



US009557669B2

(12) **United States Patent**  
Nagai et al.

(10) **Patent No.:** US 9,557,669 B2  
(45) **Date of Patent:** Jan. 31, 2017

(54) **TONER, DEVELOPER, AND IMAGE FORMING APPARATUS**

(71) Applicants: **Shinsuke Nagai**, Shizuoka (JP); **Shinya Nakayama**, Shizuoka (JP); **Tsuyoshi Sugimoto**, Shizuoka (JP); **Susumu Chiba**, Shizuoka (JP); **Kohsuke Nagata**, Shizuoka (JP); **Daisuke Asahina**, Shizuoka (JP)

(72) Inventors: **Shinsuke Nagai**, Shizuoka (JP); **Shinya Nakayama**, Shizuoka (JP); **Tsuyoshi Sugimoto**, Shizuoka (JP); **Susumu Chiba**, Shizuoka (JP); **Kohsuke Nagata**, Shizuoka (JP); **Daisuke Asahina**, Shizuoka (JP)

(73) Assignee: **Ricoh Company, Ltd.**, Tokyo (JP)

(\*) Notice: Subject to any disclaimer, the term of this patent is extended or adjusted under 35 U.S.C. 154(b) by 0 days.

(21) Appl. No.: **14/916,911**

(22) PCT Filed: **Aug. 29, 2014**

(86) PCT No.: **PCT/JP2014/073417**

§ 371 (c)(1),  
(2) Date: **Mar. 4, 2016**

(87) PCT Pub. No.: **WO2015/034028**

PCT Pub. Date: **Mar. 12, 2015**

(65) **Prior Publication Data**

US 2016/0231661 A1 Aug. 11, 2016

(30) **Foreign Application Priority Data**

Sep. 6, 2013 (JP) ..... 2013-185194

(51) **Int. Cl.**

**G03G 9/08** (2006.01)

**G03G 15/08** (2006.01)

**G03G 9/087** (2006.01)

(52) **U.S. Cl.**

CPC ..... **G03G 9/0821** (2013.01); **G03G 9/08755** (2013.01); **G03G 9/08764** (2013.01);  
(Continued)

(58) **Field of Classification Search**

CPC .. **G03G 15/08**; **G03G 9/0821**; **G03G 9/08755**; **G03G 9/08791**; **G03G 9/08764**; **G03G 9/08795**; **G03G 9/08797**  
(Continued)

(56) **References Cited**

U.S. PATENT DOCUMENTS

5,955,234 A 9/1999 Matsunaga et al.  
7,261,989 B2 8/2007 Sugiura et al.  
(Continued)

FOREIGN PATENT DOCUMENTS

EP 1 995 639 A1 11/2008  
EP 2 562 202 A1 2/2013  
(Continued)

OTHER PUBLICATIONS

International Search Report Issued Oct. 14, 2014 for counterpart International Patent Application No. PCT/JP2014/073417 filed Aug. 29, 2014.

(Continued)

*Primary Examiner* — Sophia S Chen

(74) *Attorney, Agent, or Firm* — Oblon, McClelland, Maier & Neustadt, L.L.P.

(57) **ABSTRACT**

A toner, wherein the toner has glass transition temperature [Tg1st (toner)] of 20° C. to 50° C., where the glass transition temperature [Tg1st (toner)] is measured in a first heating in differential scanning calorimetry (DSC) of the toner,

(Continued)



wherein tetrahydrofuran (THF) insoluble matter of the toner has glass transition temperature [Tg2nd (THF insoluble matter)] of -40° C. to 30° C., where the glass transition temperature [Tg2nd (THF insoluble matter)] is measured in a second heating in differential scanning calorimetry (DSC) of the tetrahydrofuran (THF) insoluble matter, wherein the THF insoluble matter has a storage modulus at 100° C. [G'(100) (THF insoluble matter)] of 1.0×10<sup>5</sup> Pa to 1.0×10<sup>7</sup> Pa, and wherein a ratio of a storage modulus of the THF insoluble matter at 40° C. [G'(40) (THF insoluble matter)] to the storage modulus of the THF insoluble matter at 100° C. [G'(100) (THF insoluble matter)] is 3.5×10 or less.

### 10 Claims, 4 Drawing Sheets

#### (52) U.S. Cl.

CPC ..... **G03G 9/08791** (2013.01); **G03G 9/08795** (2013.01); **G03G 9/08797** (2013.01); **G03G 15/08** (2013.01)

#### (58) Field of Classification Search

USPC ..... 399/252; 430/105, 108.1, 109.1  
See application file for complete search history.

#### (56) References Cited

##### U.S. PATENT DOCUMENTS

|                 |         |                   |
|-----------------|---------|-------------------|
| 7,318,989 B2    | 1/2008  | Kotsugai et al.   |
| 7,455,942 B2    | 11/2008 | Nagatomo et al.   |
| 8,673,528 B2    | 3/2014  | Sugimoto et al.   |
| 2004/0072091 A1 | 4/2004  | Mochizuki et al.  |
| 2004/0115550 A1 | 6/2004  | Sugiura et al.    |
| 2004/0229148 A1 | 11/2004 | Kadota et al.     |
| 2005/0026064 A1 | 2/2005  | Sugiura et al.    |
| 2005/0089786 A1 | 4/2005  | Sugiura et al.    |
| 2005/0089787 A1 | 4/2005  | Uchinokura et al. |
| 2005/0208408 A1 | 9/2005  | Uchinokura et al. |
| 2006/0029433 A1 | 2/2006  | Saito et al.      |
| 2006/0040197 A1 | 2/2006  | Kabai             |
| 2008/0014527 A1 | 1/2008  | Kotsugai et al.   |
| 2008/0070151 A1 | 3/2008  | Sugimoto et al.   |
| 2008/0118855 A1 | 5/2008  | Nakayama et al.   |
| 2008/0227002 A1 | 9/2008  | Moriya et al.     |
| 2008/0261131 A1 | 10/2008 | Nakayama et al.   |
| 2008/0280218 A1 | 11/2008 | Sabu et al.       |
| 2008/0280219 A1 | 11/2008 | Nakayama et al.   |
| 2008/0318143 A1 | 12/2008 | Nakayama et al.   |
| 2008/0318144 A1 | 12/2008 | Watanabe et al.   |
| 2008/0318148 A1 | 12/2008 | Sugimoto et al.   |
| 2009/0011356 A1 | 1/2009  | Tomita et al.     |
| 2009/0074467 A1 | 3/2009  | Seshita et al.    |
| 2009/0092917 A1 | 4/2009  | Sugimoto et al.   |
| 2009/0104555 A1 | 4/2009  | Wakamatsu et al.  |
| 2009/0214973 A1 | 8/2009  | Sugimoto et al.   |
| 2009/0325099 A1 | 12/2009 | Watanabe et al.   |
| 2010/0035170 A1 | 2/2010  | Sugimoto et al.   |

|                  |         |                                      |
|------------------|---------|--------------------------------------|
| 2011/0281213 A1  | 11/2011 | Sakashita et al.                     |
| 2012/0064447 A1  | 3/2012  | Hozumi et al.                        |
| 2012/0065357 A1  | 3/2012  | Yamauchi et al.                      |
| 2012/0082926 A1  | 4/2012  | Suzuki et al.                        |
| 2012/0282000 A1  | 11/2012 | Nakayama et al.                      |
| 2012/0295193 A1  | 11/2012 | Hanatani et al.                      |
| 2013/0041125 A1  | 2/2013  | Hishida et al.                       |
| 2013/0045442 A1  | 2/2013  | Moriya et al.                        |
| 2013/0059247 A1  | 3/2013  | Sugimoto et al.                      |
| 2013/0078563 A1  | 3/2013  | Nakayama et al.                      |
| 2013/0095422 A1  | 4/2013  | Yamamoto et al.                      |
| 2013/0108950 A1  | 5/2013  | Yamamoto et al.                      |
| 2013/0115550 A1  | 5/2013  | Amemori et al.                       |
| 2013/0143155 A1  | 6/2013  | Santo et al.                         |
| 2013/0157183 A1  | 6/2013  | Santo et al.                         |
| 2013/0157184 A1  | 6/2013  | Sugimoto et al.                      |
| 2013/0157185 A1  | 6/2013  | Sakashita et al.                     |
| 2013/0157193 A1  | 6/2013  | Moritani et al.                      |
| 2013/0236826 A1  | 9/2013  | Makabe et al.                        |
| 2013/0244011 A1  | 9/2013  | Sabu et al.                          |
| 2013/0244153 A1  | 9/2013  | Nakayama et al.                      |
| 2013/0244154 A1  | 9/2013  | Yamamoto et al.                      |
| 2013/0244168 A1  | 9/2013  | Yamashita et al.                     |
| 2013/0252158 A1  | 9/2013  | Yamada et al.                        |
| 2013/0260298 A1  | 10/2013 | Amemori et al.                       |
| 2013/0337374 A1  | 12/2013 | Sugimoto et al.                      |
| 2014/0023965 A1  | 1/2014  | Chiba et al.                         |
| 2014/0051019 A1  | 2/2014  | Sekiguchi et al.                     |
| 2014/0065534 A1  | 3/2014  | Amemori et al.                       |
| 2014/0080046 A1  | 3/2014  | Asahina et al.                       |
| 2014/0080050 A1  | 3/2014  | Asahina et al.                       |
| 2014/0270874 A1  | 9/2014  | Hase et al.                          |
| 2014/0272689 A1  | 9/2014  | Yamashita et al.                     |
| 2014/0301757 A1  | 10/2014 | Sakashita et al.                     |
| 2015/0248070 A1* | 9/2015  | Chiba ..... G03G 9/08755<br>430/105  |
| 2015/0378272 A1* | 12/2015 | Hase ..... G03G 9/08755<br>430/109.4 |

##### FOREIGN PATENT DOCUMENTS

|    |             |         |
|----|-------------|---------|
| JP | 2579150     | 11/1996 |
| JP | 10-171156   | 6/1998  |
| JP | 11-133665   | 5/1999  |
| JP | 2001-158819 | 6/2001  |
| JP | 2002-287400 | 10/2002 |
| JP | 2002-351143 | 12/2002 |
| JP | 2004-046095 | 2/2004  |
| JP | 2004-264495 | 9/2004  |
| JP | 2006-058652 | 3/2006  |
| JP | 2006-349894 | 12/2006 |
| JP | 2007-271789 | 10/2007 |
| JP | 2013-050629 | 3/2013  |
| JP | 2013-054178 | 3/2013  |
| JP | 2013-145362 | 7/2013  |

##### OTHER PUBLICATIONS

Extended European Search Report issued Jun. 29. 2016 in Patent Application No. 14842710.7.

\* cited by examiner

FIG. 1



FIG. 2



FIG. 3



FIG. 4



FIG. 5



## 1

## TONER, DEVELOPER, AND IMAGE FORMING APPARATUS

## TECHNICAL FIELD

The present invention relates to a toner, a developer, and an image forming apparatus.

## BACKGROUND ART

In recent years, toners have been desired to have small particles size and hot offset resistance for giving high quality output images, low temperature fixing ability for energy saving, and heat resistant storage stability for resisting high-temperature, high-humidity environments during storage or transport after production. Particularly, low temperature fixing ability is very important quality of a toner, as power consumption for fixing occupies a large part in the power consumption for an entire image forming process.

Conventionally, toners produced by a kneading and pulverizing method have been used. The toner produced by the kneading and pulverizing method have problems that it is difficult to reduce the particle size thereof, and shapes of particles are uneven and a particle diameter distribution thereof is broad, which result in unsatisfactory quality of output images, and a large quantity of energy is required for fixing such toner. In the case where wax (i.e., a releasing agent) is added to the toner for improving fixing ability, moreover, the toner produced by the kneading and pulverizing method contains a large amount of the wax present near toner surfaces, as a kneaded product is cracked from an interface of wax during pulverizing. As a result of this, a releasing effect is exhibited, but on the other hand, the toner tends to cause toner deposition (i.e., filming) on a carrier, a photoconductor, and a blade. Therefore, such toner is not satisfactory in view of its characteristics on the whole.

To encounter the aforementioned problems associated with the kneading and pulverizing method, a production method of a toner in accordance with a polymerization method has been proposed. A toner produced by the polymerization method is easily produced as small particles, has a sharp particle diameter distribution compared to that of the toner produced by the pulverizing method, and can encapsulate a releasing agent therein. As a production method of a toner in accordance with the polymerization method, proposed is a method for producing a toner using an elongation reaction product of urethane-modified polyester as a toner binder, for the purpose of improving low temperature fixing ability, and hot offset resistance (see PTL 1).

Moreover, proposed is a production method of a toner, which is excellent in all of heat resistant storage stability, low temperature fixing ability, and hot offset resistance, as well as excellent in powder flowability and transfer ability, when a toner is produced as a small-diameter toner (see PTLs 2 and 3).

Further, disclosed is a production method of a toner having a maturing step for producing a toner binder having a stable molecular weight distribution, and achieving both low temperature fixing ability and (see PTLs 4 and 5).

However, these proposed techniques do not provide a toner having a high level of low temperature fixing ability, which has been demanded in recent years.

For the purpose of achieving a high level of low temperature fixing ability, therefore, proposed is a toner containing a resin including a crystalline polyester resin, and a releasing agent, and having a phase separation structure,

## 2

where the resin and the releasing agent (e.g., wax) are incompatible to each other in the form of sea-islands (see PTL 6).

Moreover, proposed is a toner containing a crystalline polyester resin, a releasing agent, and a graft polymer (see PTL 7).

These proposed techniques can achieve low temperature fixing, as the crystalline polyester resin is rapidly melted, compared to a non-crystalline polyester resin. However, in the case of a toner containing a crystalline polyester resin, there is a problem that aggregates of the toner form in a high-temperature, high-humidity environment.

Also, although the recent demands for further improvements in qualities have required toners to be excellent not only in low temperature fixing ability and heat resistant storage stability but also in image gloss, such toners have not been obtained.

Under such circumstances, there is currently a demand for a toner excellent not only in low temperature fixing ability and heat resistant storage stability but also in image gloss.

## CITATION LIST

## Patent Literature

- PTL 1: Japanese Patent Application Laid-Open (JP-A) No. 11-133665  
 PTL 2: JP-A No. 2002-287400  
 PTL 3: JP-A No. 2002-351143  
 PTL 4: Japanese Patent (JP-B) No. 2579150  
 PTL 5: JP-A No. 2001-158819  
 PTL 6: JP-A No. 2004-46095  
 PTL 7: JP-A No. 2007-271789

## SUMMARY OF INVENTION

## Technical Problem

The present invention aims to solve the above existing problems and achieve the following object; i.e., providing a toner excellent not only in low temperature fixing ability and heat resistant storage stability but also in image gloss.

## Solution to Problem

Means for solving the above problems are as follows.

That is, a toner of the present invention has a glass transition temperature [Tg1st (toner)] of 20° C. to 50° C., where the glass transition temperature [Tg1st (toner)] is measured in a first heating in differential scanning calorimetry (DSC) of the toner,

wherein tetrahydrofuran (THF) insoluble matter of the toner has a glass transition temperature [Tg2nd (THF insoluble matter)] of -40° C. to 30° C., where the glass transition temperature [Tg2nd (THF insoluble matter)] is measured in a second heating in differential scanning calorimetry (DSC) of the tetrahydrofuran (THF) insoluble matter,

wherein the THF insoluble matter has a storage modulus at 100° C. [G'(100) (THF insoluble matter)] of  $1.0 \times 10^5$  Pa to  $1.0 \times 10^7$  Pa, and

wherein a ratio of a storage modulus of the THF insoluble matter at 40° C. [G'(40) (THF insoluble matter)] to the storage modulus of the THF insoluble matter at 100° C. [G'(100) (THF insoluble matter)], expressed by  $[[G'(40) (THF insoluble matter)]/[G'(100) (THF insoluble matter)]]$ , is  $3.5 \times 10$  or less.

## Advantageous Effects of Invention

The present invention can solve the above existing problems and provide a toner excellent not only in low temperature fixing ability and heat resistant storage stability but also in image gloss.

## BRIEF DESCRIPTION OF DRAWINGS

FIG. 1 is a schematic structural view of one example of an image forming apparatus of the present invention.

FIG. 2 is a schematic structural view of another example of an image forming apparatus of the present invention.

FIG. 3 is a schematic structural view of still another example of an image forming apparatus of the present invention.

FIG. 4 is a partially enlarged view of FIG. 3.

FIG. 5 is a schematic structural view of one example of a process cartridge.

## DESCRIPTION OF EMBODIMENTS

## Toner

A toner of the present invention has a glass transition temperature [Tg1st (toner)] of 20° C. to 50° C., where the glass transition temperature [Tg1st (toner)] is measured in a first heating in differential scanning calorimetry (DSC) of the toner.

Tetrahydrofuran (THF) insoluble matter of the toner has a glass transition temperature [Tg2nd (THF insoluble matter)] of -40° C. to 30° C., where the glass transition temperature [Tg2nd (THF insoluble matter)] is measured in a second heating in differential scanning calorimetry (DSC) of the tetrahydrofuran (THF) insoluble matter.

The THF insoluble matter has a storage modulus at 100° C. [G'(100) (THF insoluble matter)] of  $1.0 \times 10^5$  Pa to  $1.0 \times 10^7$  Pa.

A ratio of a storage modulus of the THF insoluble matter at 40° C. [G'(40) (THF insoluble matter)] to the storage modulus of the THF insoluble matter at 100° C. [G'(100) (THF insoluble matter)], expressed by  $[[G'(40) (THF insoluble matter)]/[G'(100) (THF insoluble matter)]]$ , is 3.5×10 or less.

The values of the [Tg2nd (THF insoluble matter)], the [G'(100) (THF insoluble matter)] and the [G'(40) (THF insoluble matter)] can be adjusted by adjusting a resin composition (a dihydric or higher polyol, a divalent or higher acid component), for example.

Specifically, these values can be adjusted in the following manner, for example.

For lowering the Tg, a polyol containing an alkyl group in a side chain thereof is used as a constituent component of a resin.

For increasing the Tg, the distance between ester bonds in the resin is shortened.

For increasing the G', the distance between ester bonds in the resin is shortened and a resin composition containing an aromatic compound is used.

For lowering the G', a linear chain polyester resin is used and a polyol containing an alkyl group in a side chain thereof is used as a constituent component of a resin.

## &lt;THF Insoluble Matter&gt;

The tetrahydrofuran (THF) insoluble matter of the toner is not particularly limited and may be appropriately selected depending on the intended purpose, but it is preferably 15% by mass to 35% by mass, more preferably 20% by mass to

30% by mass. When the THF insoluble matter is less than 15% by mass, the toner may be degraded in low temperature fixing ability. When the THF insoluble matter is more than 35% by mass, the toner may be degraded in heat resistant storage stability.

The THF insoluble matter corresponds to a non-linear chain non-crystalline polyester resin. Although the toner of the present invention has a lower Tg than that of conventional toners, the toner of the present invention can retain sufficient heat resistant storage stability since it contains the THF insoluble matter in a specific amount. Especially in the case where the non-crystalline polyester resin has a urethane bond or a urea bond having high cohesive force, an effect of maintaining heat resistant storage stability will become more significant.

## &lt;THF Insoluble Matter and THF Soluble Matter&gt;

The THF soluble matter of the toner and the THF insoluble matter of the toner can be obtained in the following manner.

A toner (1 part by mass) is added to 40 parts by mass of tetrahydrofuran (THF) and the mixture is refluxed for 6 hours. Thereafter, insoluble components are made to sediment with a centrifugal device, to thereby be separated from a supernatant.

The insoluble components are dried at 40° C. for 20 hours to obtain the THF insoluble matter.

The solvent is removed from the above-separated supernatant, followed by drying at 40° C. for 20 hours, to thereby obtain the THF soluble matter.

## &lt;Glass Transition Temperature&gt;

## &lt;&lt;[Tg1st (Toner)]&gt;&gt;

The toner has a glass transition temperature (Tg1st) of 20° C. to 50° C., preferably 35° C. to 45° C., where the glass transition temperature (Tg1st) is measured in the first heating in differential scanning calorimetry (DSC) of the toner.

If the Tg of a conventional toner is lowered to be about 50° C. or lower, the conventional toner tends to cause aggregation of toner particles influenced by temperature variations during transportation or storage of the toner in summer or in a tropical region. As a result, adherence of the toner occurs in a toner bottle, or within a developing unit. Moreover, supply failures due to clogging of the toner in the toner bottle, and formation of defected images due to toner adherence are likely to occur.

The toner of the present invention has lower Tg than that of a conventional toner. However, the toner of the present invention can maintain heat resistant storage stability. Especially in the case where the non-crystalline polyester resin has a urethane bond or a urea bond having high cohesive force, an effect of maintaining heat resistant storage stability will become more significant.

When the [Tg1st (toner)] is lower than 20° C., degradation in heat resistant storage stability, blocking in developing devices, and filming to a photoconductor will arise. When the [Tg1st (toner)] is higher than 50° C., the toner will be degraded in low temperature fixing ability.

## &lt;&lt;[Tg2nd (Toner)]&gt;&gt;

The glass transition temperature [Tg2nd (toner)] of the toner measured in a second heating in differential scanning calorimetry (DSC) of the toner is not particularly limited and may be appropriately selected depending on the intended purpose, but it is preferably 0° C. to 30° C., more preferably 15° C. to 30° C.

When the [Tg2nd (toner)] is lower than 0° C., blocking resistance of a fixed image (printed matter) may be

degraded. When the [Tg2nd (toner)] is higher than 30° C., it may be impossible to attain sufficient low temperature fixing ability and glossiness.

The value of the [Tg2nd (toner)] can be adjusted by adjusting the Tg and the amount of the crystalline polyester resin, for example.

<<[Tg1st (toner)]-[Tg2nd (toner)]>>

A difference ([Tg1st (toner)]-[Tg2nd (toner)]) between the glass transition temperature [Tg1st (toner)] of the toner as measured in the first heating in differential scanning calorimetry (DSC) and the glass transition temperature [Tg2nd (toner)] of the toner as measured in the second heating in DSC is not particularly limited and may be appropriately selected depending on the intended purpose, but it is preferably 10° C. or more. The upper limit of the difference is not particularly limited and may be appropriately selected depending on the intended purpose, but the difference ([Tg1st (toner)]-[Tg2nd (toner)]) is preferably 50° C. or less.

When the difference ([Tg1st (toner)]-[Tg2nd (toner)]) is 10° C. or more, the resultant toner is excellent in low temperature fixing ability, which is advantageous. The fact that the difference ([Tg1st (toner)]-[Tg2nd (toner)]) is 10° C. or more means that the crystalline polyester resin and the non-crystalline polyester resin, which are present in a non-compatible state before heating (before the first heating), become in a compatible state after heating (after the first heating). Note that, the compatible state after heating does not have to be a completely compatible state.

<<[Tg2nd (THF Insoluble Matter)]>>

A glass transition temperature [Tg2nd (THF insoluble matter)] of the THF insoluble matter of the toner, which is measured in a second heating in differential scanning calorimetry (DSC), is -40° C. to 30° C., preferably 0° C. to 20° C.

When the glass transition temperature [Tg2nd (THF insoluble matter)] is lower than -40° C., the heat resistant storage stability will be degraded. When the glass transition temperature [Tg2nd (THF insoluble matter)] is higher than 30° C., the low temperature fixing property will be degraded.

The glass transition temperature [Tg2nd (THF insoluble matter)] corresponds to Tg2nd of the non-linear chain non-crystalline polyester resin, and the above range of the glass transition temperature [Tg2nd (THF insoluble matter)] is advantageous for low temperature fixing ability. Also, when the non-linear chain, non-crystalline polyester resin has a urethane bond or a urea bond having high cohesive force, an effect of maintaining heat resistant storage stability will become more significant.

<<[Tg2nd (THF Soluble Matter)]>>

A glass transition temperature [Tg2nd (THF soluble matter)] of the THF soluble matter of the toner, which is measured in a second heating in differential scanning calorimetry (DSC), is preferably 5° C. to 35° C., more preferably 25° C. to 35° C.

The THF soluble matter of the toner is usually composed of a crystalline polyester resin and a non-crystalline polyester resin which is a component having a high Tg. The crystalline polyester resin exhibits thermofusion characteristics in which viscosity is drastically decreases at temperature around fixing onset temperature, as the crystalline polyester resin has crystallinity. By using the crystalline polyester resin having the aforementioned characteristics together with the non-crystalline polyester resin in the toner, the heat resistant storage stability of the toner is excellent up to the melt onset temperature owing to crystallinity, and the toner drastically decreases its viscosity at the melt onset

temperature because of melting of the crystalline polyester resin. Along with the drastic decrease in viscosity, the crystalline polyester resin is melt together with the non-crystalline polyester resin, to drastically decrease their viscosity to thereby be fixed. Accordingly, a toner having excellent heat resistant storage stability and low temperature fixing ability can be obtained. Moreover, the toner has excellent results in terms of a releasing width (a difference between the minimum fixing temperature and hot offset occurring temperature).

The value of the [Tg2nd (THF soluble matter)] can be adjusted by adjusting the Tg of the non-crystalline polyester resin, the Tg of the crystalline polyester resin, and the amounts of the non-crystalline polyester resin and the crystalline polyester resin.

<<Storage Modulus>>

<<[G'(100) (THF Insoluble Matter)] and [[G'(40) (THF Insoluble Matter)]/[G'(100) (THF Insoluble Matter)]]>>

The THF insoluble matter of the toner preferably has a storage modulus at 100° C. [G'(100) (THF insoluble matter)] of  $1.0 \times 10^5$  Pa to  $1.0 \times 10^7$  Pa, preferably  $5.0 \times 10^5$  Pa to  $5.0 \times 10^6$  Pa.

The ratio of a storage modulus of the THF insoluble matter of the toner at 40° C. [G'(40) (THF insoluble matter)] to the storage modulus of the THF insoluble matter of the toner at 100° C. [G'(100) (THF insoluble matter)], expressed by [[G'(40) (THF insoluble matter)]/[G'(100) (THF insoluble matter)]], is  $3.5 \times 10$  or less, preferably  $3.3 \times 10$  or less. The lower limit of the ratio [[G'(40) (THF insoluble matter)]/[G'(100) (THF insoluble matter)]] is not particularly limited and may be appropriately selected depending on the intended purpose, but the ratio [[G'(40) (THF insoluble matter)]/[G'(100) (THF insoluble matter)]] is preferably  $2.0 \times 10$  or more.

When the toner has the [G'(100) (THF insoluble matter)] of  $1.0 \times 10^5$  Pa to  $1.0 \times 10^7$  Pa and the ratio [[G'(40) (THF insoluble matter)]/[G'(100) (THF insoluble matter)]] of  $3.5 \times 10$  or less, the crystalline polyester resin is melt more together with the non-crystalline polyester resin which is a component having a high Tg. As a result, the  $\frac{1}{2}$  outflow onset temperature measured with a thermal flow evaluating device (flow tester) will decrease and image gloss will improve.

<<[G'(100) (Toner)]>>

The toner has a storage modulus at 100° C. [G'(100) (toner)] of  $5.0 \times 10^3$  Pa to  $5.0 \times 10^4$  Pa. When the [G'(100) (toner)] is less than  $5.0 \times 10^3$  Pa, hot offset may occur. When the [G'(100) (toner)] is more than  $5.0 \times 10^4$  Pa, the minimum fixing temperature may increase.

The value of the [G'(100) (toner)] can be adjusted by adjusting the composition of the non-linear chain, non-crystalline polyester resin, for example,

<<Measurement Method of Storage Modulus G'>>

The storage modulus (G') under various conditions can be measured using, for example, a dynamic viscoelasticity measuring device (ARES, product of TA Instruments, Inc.). A frequency in the measurement is 1 Hz.

Specifically, a measurement sample is formed into a pellet having a diameter of 8 mm and a thickness of 1 mm to 2 mm, fixed on a parallel plate having a diameter of 8 mm, which is then stabilized at 40° C., and heated to 200° C. at a heating rate of 2.0° C./min with a frequency of 1 Hz (6.28 rad/s) and a strain amount of 0.1% (strain amount control mode), and a storage modulus is measured.

In the present specification, the storage modulus at 40° C. may be referred to as G'(40° C.) and the storage modulus at 100° C. may be referred to as G'(100° C.).

## &lt;Melting Point&gt;

The melting point of the toner is not particularly limited and may be appropriately selected depending on the intended purpose, but it is preferably 60° C. to 80° C.

## &lt;Volume Average Particle Diameter&gt;

The volume average particle diameter of the toner is not particularly limited and may be appropriately selected depending on the intended purpose, but it is preferably 3 µm to 7 µm. Moreover, a ratio of the volume average particle diameter to the number average particle diameter is preferably 1.2 or less. Further, the toner preferably contains toner particles having the volume average particle diameter of 2 m or smaller, in an amount of 1% by number to 10% by number.

## &lt;Calculation Methods and Analysis Methods of Various Properties of Toner and Constituent Component of Toner&gt;

The Tg, acid value, hydroxyl value, molecular weight, and melting point of the polyester resin and the releasing agent may be each measured. Alternatively, each component may be separated from an actual toner by gel permeation chromatography (GPC) or the like, and separated each component may be subjected to the analysis methods described later, to thereby calculate Tg, molecular weight, melting point, and mass ratio of a constituent component.

Separation of each component by GPC can be performed, for example, by the following method.

In GPC using tetrahydrofuran (THF) as a mobile phase, an eluate is subjected to fractionation by means of a fraction collector, a fraction corresponding to a part of a desired molecular weight is collected from a total area of an elution curve.

The collected eluates are concentrated and dried by an evaporator or the like, and a resulting solid content is dissolved in a deuterated solvent, such as deuterated chloroform, and deuterated THF, followed by measurement of <sup>1</sup>H-NMR. From an integral ratio of each element, a ratio of a constituent monomer of the resin in the elution composition is calculated.

As another method, after concentrating the eluate, hydrolysis is performed with sodium hydroxide or the like, and a ratio of a constituent monomer is calculated by subjecting the decomposed product to a qualitative or quantitative analysis by high performance liquid chromatography (HPLC).

Note that, in the case where the method for producing a toner produces toner base particles by generating the non-crystalline polyester resin through a chain-elongation reaction and/or crosslink reaction of the non-linear chain reactive precursor and the curing agent, the polyester resin may be separated from an actual toner by GPC or the like, to thereby determine Tg thereof. Alternatively, a non-crystalline polyester resin is separately generated through a chain-elongation reaction and/or crosslink reaction of the non-linear chain reactive precursor and the curing agent, and Tg may be measured on the synthesized non-crystalline polyester resin.

## &lt;&lt;Separation Unit for Toner Constituent Components&gt;&gt;

An example of a separation unit for each component during an analysis of the toner will be specifically explained hereinafter.

First, 1 g of a toner is added to 100 mL THF, and the resulting mixture is stirred for 30 minutes at 25° C., to thereby a solution in which soluble components are dissolved.

The solution is then filtered through a membrane filter having an opening of 0.2 µm, to thereby obtain the THF soluble components in the toner.

Next, the THF soluble components are dissolved in THF, to thereby prepare a sample for measurement of GPC, and the prepared sample is supplied to GPC used for molecular weight measurement of each resin mentioned above.

Meanwhile, a fraction collector is disposed at an eluate outlet of GPC, to fraction the eluate per a certain count. The eluate is obtained per 5% in terms of the area ratio from the elution onset on the elution curve (raise of the curve).

Next, each eluted fraction, as a sample, in an amount of 10 30 mg is dissolved in 1 mL of deuterated chloroform, and to this solution, 0.05% by volume of tetramethyl silane (TMS) is added as a standard material.

A glass tube for NMR having a diameter of 5 mm is charged with the solution, from which a spectrum is obtained by means of a nuclear magnetic resonance apparatus (JNM-AL 400, manufactured by JEOL Ltd.) by performing multiplication 128 times at temperature of 23° C. to 25° C.

The monomer compositions and the compositional ratios of the non-crystalline polyester resin, the crystalline polyester resin, and the like contained in the toner are determined from peak integral ratios of the obtained spectrum.

For example, an assignment of a peak is performed in the following manner, and a constituent monomer component ratio is determined from each integral ratio.

The assignment of a peak is as follows:

Around 8.25 ppm: derived from a benzene ring of trimellitic acid (for one hydrogen atom)

Around the region of 8.07 ppm to 8.10 ppm: derived from a benzene ring of terephthalic acid (for four hydrogen atoms)

Around the region of 7.1 ppm to 7.25 ppm: derived from a benzene ring of bisphenol A (for four hydrogen atoms)

Around 6.8 ppm: derived from a benzene ring of bisphenol A (for four hydrogen atoms), and derived from a double bond of fumaric acid (for two hydrogen atoms)

Around the region of 5.2 ppm to 5.4 ppm: derived from methine of bisphenol A propylene oxide adduct (for one hydrogen atom)

Around the region of 3.7 ppm to 4.7 ppm: derived from methylene of a bisphenol A propylene oxide adduct (for two hydrogen atoms), and derived from methylene of a bisphenol A ethylene oxide (for four hydrogen atoms)

Around 1.6 ppm: derived from a methyl group of bisphenol A (for 6 hydrogen atoms).

From these results, for example, the extracted product collected in the fraction in which the non-crystalline polyester resin occupies 90% or more in the peak integral ratio in the spectrum can be treated as the non-crystalline polyester resin.

Similarly, the extracted product collected in the fraction in which the crystalline polyester resin occupies 90% or more in the peak integral ratio in the spectrum can be treated as the crystalline polyester resin.

## &lt;&lt;Measurement Methods of Melting Point and Glass Transition Temperature (Tg)&gt;&gt;

In the present invention, a melting point and a glass transition temperature (Tg) can be measured, for example, by means of a differential scanning calorimeter (DSC) system (Q-200, manufactured by TA Instruments Japan Inc.).

Specifically, a melting point and glass transition temperature of a sample are measured in the following manners.

Specifically, first, an aluminum sample container charged with about 5.0 mg of a sample is placed on a holder unit, and the holder unit is then set in an electric furnace. Next, the sample is heated (first heating) from -80° C. to 150° C. at

the heating rate of 10° C./min in a nitrogen atmosphere. Then, the sample is cooled from 150° C. to -80° C. at the cooling rate of 10° C./min, followed by again heating (second heating) to 150° C. at the heating rate of 10° C./min. DSC curves are respectively measured for the first heating and the second heating by means of a differential scanning calorimeter (Q-200, manufactured by TA Instruments Japan Inc.).

The DSC curve for the first heating is selected from the obtained DSC curve by means of an analysis program stored in the Q-200 system, to thereby determine glass transition temperature of the sample with the first heating. Similarly, the DSC curve for the second heating is selected, and the glass transition temperature of the sample with the second heating can be determined.

Moreover, the DSC curve for the first heating is selected from the obtained DSC curve by means of the analysis program stored in the Q-200 system, and an endothermic peak top temperature of the sample for the first heating is determined as a melting point of the sample. Similarly, the DSC curve for the second heating is selected, and the endothermic peak top temperature of the sample for the second heating can be determined as a melting point of the sample with the second heating.

In the case where a toner is used as a sample, glass transition temperature for the first heating is represented as Tg1st, and glass transition temperature for the second heating is represented as Tg2nd in the present specification.

Moreover, in the present specification, the endothermic peak top temperatures and glass transition temperatures of the non-crystalline polyester resin, the crystalline polyester resin, and other constituent components, such as the releasing agent, for the second heating are regarded as melting point and Tg of each sample, unless otherwise stated.

The toner preferably contains a polyester resin.

<Polyester Resin>

The polyester resin is not particularly limited and may be appropriately selected depending on the intended purpose, but it preferably contains a non-crystalline polyester resin and crystalline polyester resin C.

The non-crystalline polyester resin contains a dicarboxylic acid component as a constituent component, and the dicarboxylic acid component preferably contains terephthalic acid in an amount of 50 mol % or more, which is advantageous in terms of heat resistant storage stability.

Also, the polyester resin preferably contains non-crystalline polyester resin A, non-crystalline polyester resin B, and the crystalline polyester resin C.

The non-crystalline polyester resin A is preferably obtained through reaction between a non-linear reactive precursor and a curing agent.

The non-crystalline polyester resin A preferably has a glass transition temperature of -60° C. to 0° C.

The non-crystalline polyester resin B preferably has a glass transition temperature of 40° C. to 80° C.

One conceivable method for improving low temperature fixing ability of a toner is lowering the glass transition temperature or the molecular weight of a non-crystalline polyester resin so that the non-crystalline polyester resin melt with a crystalline polyester resin. However, it can easily be imagined that when simply lowering the glass transition temperature or the molecular weight of the non-crystalline polyester resin to lower its melt viscosity, the resultant toner will be degraded in heat resistant storage stability and hot offset resistance upon fixing.

In the toner of the present invention, the non-crystalline polyester resin A has a very low glass transition temperature

and has a property of deforming at low temperature. Hence, the non-crystalline polyester resin A has such a property that it deforms with heating and pressing upon fixing and easily adheres on recording media such as paper at low temperature. Also, since a reactive precursor of the non-crystalline polyester resin A is a non-linear chain, the non-crystalline polyester resin A has a branched structure in its molecular skeleton, and the molecular chain thereof becomes a three-dimensional network structure. As a result, the non-crystalline polyester resin A has such rubber-like properties as to deform at low temperature but not flow, enabling the toner to retain heat resistant storage stability and hot offset resistance. Note that, when the non-crystalline polyester resin A has a urethane bond or a urea bond having high cohesive energy, the obtained toner is more excellent in adhesion onto recording media such as paper. Also, the urethane bond or the urea bond behaves as a pseudo-crosslinking point to increase rubber-like properties of the polyester resin. As a result, the obtained toner is more excellent in heat resistant storage stability and hot offset resistance.

Specifically, in one aspect of the toner of the present invention, by combining the non-crystalline polyester resin A, which has a glass transition temperature in an ultra low temperature region but does not easily flow owing to high melt viscosity, with the non-crystalline polyester resin B and the crystalline polyester resin C, it becomes possible to maintain heat resistant storage stability and hot offset resistance even when the glass transition temperature of the toner is set to be lower than that of a conventional toner; and by making the toner have a low glass transition temperature, the toner is excellent in low temperature fixing ability.

<<Non-Crystalline Polyester Resin A>>

The non-crystalline polyester resin A is preferably obtained through reaction between a non-linear chain reactive precursor and a curing agent.

The non-crystalline polyester resin A preferably has a glass transition temperature of -60° C. to 0° C.

The non-crystalline polyester resin A preferably contains a urethane bond, a urea bond, or both, since it is more excellent in adhesion onto recording media such as paper. Also, as a result of containing a urethane bond, a urea bond, or both in the non-crystalline polyester resin A, the urethane bond or the urea bond behaves as a pseudo-crosslinking point to increase rubber-like properties of the non-crystalline polyester resin A. As a result, the obtained toner is more excellent in heat resistant storage stability and hot offset resistance.

The non-crystalline polyester resin A contains a dicarboxylic acid component as a constituent component thereof, and the dicarboxylic acid component preferably contains an aliphatic dicarboxylic acid in an amount of 60 mol % or more.

Examples of the dicarboxylic acid component include an aliphatic dicarboxylic acid having 4 to 12 carbon atoms. Examples of the aliphatic dicarboxylic acid having 4 to 12 carbon atoms include succinic acid, glutaric acid, adipic acid, pimelic acid, suberic acid, azelaic acid, sebacic acid, and decanedioic acid.

-Non-Linear Chain Reactive Precursor-

The non-linear chain reactive precursor is not particularly limited and may be appropriately selected depending on the intended purpose so long as it is a polyester resin containing a reactive group with the curing agent (hereinafter may be referred to as "prepolymer").

Examples of the reactive group with the curing agent in the prepolymer include a group reactive with an active hydrogen group. Examples of the group reactive with an

## 11

active hydrogen group include an isocyanate group, an epoxy group, carboxylic acid, and an acid chloride group. Among them, an isocyanate group is preferred since it is possible to introduce a urethane bond or a urea bond into the non-crystalline polyester resin.

The prepolymer is a non-linear chain. The non-linear chain means having a branched structure provided by a trihydric or higher alcohol, a trivalent or higher carboxylic acid, or both.

The prepolymer is preferably a polyester resin containing an isocyanate group.

## --Polyester Resin Containing an Isocyanate Group--

The polyester resin containing an isocyanate group is not particularly limited and may be appropriately selected depending on the intended purpose. Examples thereof include a reaction product between a polyisocyanate and a polyester resin containing an active hydrogen group. The polyester resin containing an active hydrogen group can be obtained, for example, through polycondensation among the following: a diol; a dicarboxylic acid; and a trihydric or higher alcohol, a trivalent or higher carboxylic acid, or both. The trihydric or higher alcohol, trivalent or higher carboxylic acid, or both provide a branched structure to the polyester resin containing an isocyanate group.

## ---Diol---

The diol not particularly limited and may be appropriately selected depending on the intended purpose. Examples thereof include aliphatic diols such as ethylene glycol, 1,2-propylene glycol, 1,3-propylene glycol, 1,4-butanediol, 3-methyl-1,5-pentanediol, 1,6-hexanediol, 1,8-octanediol, 1,10-decanediol, and 1,12-dodecanediol; diols containing an oxyalkylene group such as diethylene glycol, triethylene glycol, dipropylene glycol, polyethylene glycol, polypropylene glycol and polytetramethylene glycol; alicyclic diols such as 1,4-cyclohexanediol and hydrogenated bisphenol A; adducts of alicyclic diols with alkylene oxides such as ethylene oxide, propylene oxide, and butylene oxide; bisphenols such as bisphenol A, bisphenol F and bisphenol S; and adducts of bisphenols with alkylene oxides such as ethylene oxide, propylene oxide, and butylene oxide. Among them, aliphatic diols having 4 to 12 carbon atoms are preferred.

These diols may be used alone or in combination of two or more thereof.

## ---Dicarboxylic Acid---

The dicarboxylic acid component is not particularly limited and may be appropriately selected depending on the intended purpose. Examples thereof include aliphatic dicarboxylic acids and aromatic dicarboxylic acids. Besides, anhydrides thereof, lower (C1 to C3) alkyl-esterified compounds thereof, or halides thereof may also be used.

The aliphatic dicarboxylic acid is not particularly limited and may be appropriately selected depending on the intended purpose. Examples thereof include succinic acid, adipic acid, sebatic acid, decanedioic acid, maleic acid, and fumaric acid.

The aromatic dicarboxylic acid is not particularly limited and may be appropriately selected depending on the intended purpose, but it is preferably an aromatic dicarboxylic acid having 8 to 20 carbon atoms. The aromatic dicarboxylic acid having 8 to 20 carbon atoms is not particularly limited and may be appropriately selected depending on the intended purpose. Examples thereof include phthalic acid, isophthalic acid, terephthalic acid, and naphthalenedicarboxylic acids.

Among them, aliphatic dicarboxylic acids having 4 to 12 carbon atoms are preferred.

## 12

These dicarboxylic acids may be used alone or in combination of two or more thereof.

## ---Trihydric or Higher Alcohol---

The trihydric or higher alcohol is not particularly limited and may be appropriately selected depending on the intended purpose. Examples thereof include trihydric or higher aliphatic alcohols, trihydric or higher polyphenols, and alkylene oxide adducts of trihydric or higher polyphenols.

10 Examples of the trihydric or higher aliphatic alcohol include glycerin, trimethylethane, trimethylolpropane, pentaerythritol, and sorbitol.

Examples of the trihydric or higher polyphenols include trisphenol PA, phenol novolac, and cresol novolac.

15 Examples of the alkylene oxide adducts of trihydric or higher polyphenols include adducts of trivalent or higher polyphenols with, for example, ethylene oxide, propylene oxide, or butylene oxide.

The non-crystalline polyester resin A preferably contains 20 a trihydric or higher aliphatic alcohol as a constituent component thereof.

When the non-crystalline polyester resin A contains a trihydric or higher aliphatic alcohol as a constituent component thereof, the non-crystalline polyester resin A has a branched structure in its molecular skeleton, and the molecular chain thereof becomes a three-dimensional network structure. As a result, the non-crystalline polyester resin A has such rubber-like properties as to deform at low temperature but not flow, enabling the toner to retain heat 25 resistant storage stability and hot offset resistance.

The non-crystalline polyester resin A can also use, for example, a trivalent or higher carboxylic acid or an epoxy as the crosslink component. In this case, however, a fixed image obtained by fixing the resultant with heat may not 30 show sufficient glossiness since many trivalent or higher carboxylic acids are aromatic compounds or a density of ester bonds of the crosslink components becomes higher. Use of a crosslinking agent such as an epoxy needs crosslinking reaction after polymerization for the polyester, 35 which makes it difficult to control the distance between crosslinked points, potentially leading to failure to obtain intended viscoelasticity and/or degradation in image density or glossiness due to unevenness in the fixed image. The reason why the unevenness in the fixed image arises is that 40 the epoxy tends to react with an oligomer formed during the production of the polyester to form portions having a high crosslinked density.

## ---Trivalent or Higher Carboxylic Acid---

The trivalent or higher carboxylic acid is not particularly 45 limited and may be appropriately selected depending on the intended purpose. Examples thereof include trivalent or higher aromatic carboxylic acids. Besides, anhydrides thereof, lower (C1 to C3) alkyl-esterified compounds thereof, or halides thereof may also be used.

55 The trivalent or higher aromatic carboxylic acid is preferably a trivalent or higher aromatic carboxylic acid having 9 to 20 carbon atoms. Examples of the trivalent or higher aromatic carboxylic acid having 9 to 20 carbon atoms include trimellitic acid and pyromellitic acid.

## ---Polyisocyanate---

The polyisocyanate is not particularly limited and may be 60 appropriately selected depending on the intended purpose. Examples thereof include diisocyanate, and trivalent or higher isocyanate.

65 Examples of the diisocyanate include: aliphatic diisocyanate; alicyclic diisocyanate; aromatic diisocyanate; aromatic aliphatic diisocyanate; isocyanurate; and a block product

## 13

thereof where the foregoing compounds are blocked with a phenol derivative, oxime, or caprolactam.

The aliphatic diisocyanate is not particularly limited and may be appropriately selected depending on the intended purpose. Examples thereof include tetramethylene diisocyanate, hexamethylene diisocyanate, 2,6-diisocyanato methyl caproate, octamethylene diisocyanate, decamethylene diisocyanate, dodecamethylene diisocyanate, tetradecamethylene diisocyanate, trimethylhexane diisocyanate, and tetramethylhexane diisocyanate.

The alicyclic diisocyanate is not particularly limited and may be appropriately selected depending on the intended purpose. Examples thereof include isophorone diisocyanate, and cyclohexylmethane diisocyanate.

The aromatic diisocyanate is not particularly limited and may be appropriately selected depending on the intended purpose. Examples thereof include tolylene diisocyanate, diisocyanato diphenyl methane, 1,5-nephthylene diisocyanate, 4,4'-diisocyanato diphenyl, 4,4'-diisocyanato-3,3'-dimethylidiphenyl, 4,4'-diisocyanato-3-methylidiphenyl methane, and 4,4'-diisocyanato-diphenyl ether.

The aromatic aliphatic diisocyanate is not particularly limited and may be appropriately selected depending on the intended purpose. Examples thereof include  $\alpha,\alpha,\alpha',\alpha'$ -tetramethylxylene diisocyanate.

The isocyanurate is not particularly limited and may be appropriately selected depending on the intended purpose. Examples thereof include tris(isocyanatoalkyl)isocyanurate, and tris(isocyanatocycloalkyl)isocyanurate.

These polyisocyanates may be used alone or in combination of two or more thereof.

**-Curing Agent-**

The curing agent is not particularly limited and may be appropriately selected depending on the intended purpose so long as it can react with the non-linear reactive precursor to form the non-crystalline polyester resin A. Examples thereof include active hydrogen group-containing compounds.

**--Active Hydrogen Group-Containing Compound--**

An active hydrogen group in the active hydrogen group-containing compound is not particularly limited and may be appropriately selected depending on the intended purpose. Examples thereof include a hydroxyl group (e.g., an alcoholic hydroxyl group, and a phenolic hydroxyl group), an amino group, a carboxyl group, and a mercapto group. These may be used alone or in combination of two or more thereof.

The active hydrogen group-containing compound is not particularly limited and may be appropriately selected depending on the intended purpose, but it is preferably selected from amines, as the amines can form a urea bond.

The amines are not particularly limited and may be appropriately selected depending on the intended purpose. Examples thereof include diamine, trivalent or higher amine, amino alcohol, amino mercaptan, amino acid, and compounds in which the amino groups of the foregoing compounds are blocked. These may be used alone or in combination of two or more thereof.

Among them, diamine, and a mixture of diamine and a small amount of trivalent or higher amine are preferable.

The diamine is not particularly limited and may be appropriately selected depending on the intended purpose. Examples thereof include aromatic diamine, alicyclic diamine, and aliphatic diamine. The aromatic diamine is not particularly limited and may be appropriately selected depending on the intended purpose. Examples thereof include phenylene diamine, diethyl toluene diamine, and 4,4'-diaminodiphenyl methane. The alicyclic diamine is not particularly limited and may be appropriately selected

## 14

depending on the intended purpose. Examples thereof include 4,4'-diamino-3,3'-dimethyldicyclohexyl methane, diaminocyclohexane, and isophorone diamine. The aliphatic diamine is not particularly limited and may be appropriately selected depending on the intended purpose. Examples thereof include ethylene diamine, tetramethylene diamine, and hexamethylene diamine.

The trivalent or higher amine is not particularly limited and may be appropriately selected depending on the intended purpose. Examples thereof include diethylene triamine, and triethylene tetramine.

The amino alcohol is not particularly limited and may be appropriately selected depending on the intended purpose.

Examples thereof include ethanol amine, and hydroxyethyl amine.

The aminomercaptan is not particularly limited and may be appropriately selected depending on the intended purpose. Examples thereof include aminoethyl mercaptan, and aminopropyl mercaptan.

The amino acid is not particularly limited and may be appropriately selected depending on the intended purpose. Examples thereof include aminopropionic acid, and aminocaproic acid.

The compound where the amino group is blocked is not particularly limited and may be appropriately selected depending on the intended purpose. Examples thereof include a ketimine compound where the amino group is blocked with ketone such as acetone, methyl ethyl ketone, methyl isobutyl ketone, and an oxazoline compound.

In order to lower the Tg of the non-crystalline polyester resin A so that it is more easily provided with a property of deforming at low temperature, preferably, the non-crystalline polyester resin A contains a diol component as a constituent component thereof, and the diol component contains an aliphatic diol having 4 to 12 carbon atoms in an amount of 50% by mass or more.

In order to lower the Tg of the non-crystalline polyester resin A so that it is more easily provided with a property of deforming at low temperature, preferably, the non-crystalline polyester resin A contains the aliphatic diol having 4 to 12 carbon atoms in an amount of 50% by mass or more in all the alcohol components.

In order to lower the Tg of the non-crystalline polyester resin A so that it is more easily provided with a property of deforming at low temperature, preferably, the non-crystalline polyester resin A contains a dicarboxylic acid component as a constituent component thereof, and the dicarboxylic acid component contains an aliphatic dicarboxylic acid having 4 to 12 carbon atoms in an amount of 50% by mass or more.

A glass transition temperature of the non-crystalline polyester resin A is preferably  $-60^{\circ}\text{C}$ . to  $0^{\circ}\text{C}$ ., more preferably  $-40^{\circ}\text{C}$ . to  $-20^{\circ}\text{C}$ . When the glass transition temperature is lower than  $-60^{\circ}\text{C}$ ., the obtained toner cannot be prevented from flowing at low temperature, potentially leading to degradation in heat resistant storage stability and/or filming resistance. When the glass transition temperature thereof is higher than  $0^{\circ}\text{C}$ ., the obtained toner cannot sufficiently deform with heating and pressing upon fixing, potentially leading to insufficient low temperature fixing ability.

A weight average molecular weight of the non-crystalline polyester resin A is not particularly limited and may be appropriately selected depending on the intended purpose. It is preferably 20,000 to 1,000,000, more preferably 50,000 to 300,000, particularly preferably 100,000 to 200,000, as measured in GPC (gel permeation chromatography) measurement.

## 15

When the weight average molecular weight thereof is less than 20,000, the obtained toner more easily flows at low temperature, potentially leading to degradation in heat resistant storage stability. In addition, the toner may be degraded in hot offset resistance because of lowered viscosity of the toner upon melting.

A molecular structure of the non-crystalline polyester resin A can be confirmed by solution-state or solid-state NMR, X-ray diffraction, GC/MS, LC/MS, or IR spectroscopy. Simple methods thereof include a method for detecting, as a non-crystalline polyester resin, one that does not have absorption based on SCH (out-of-plane bending vibration) of olefin at  $965\text{ cm}^{-1}\pm10\text{ cm}^{-1}$  and  $990\text{ cm}^{-1}\pm10\text{ cm}^{-1}$  in an infrared absorption spectrum.

An amount of the non-crystalline polyester resin A is not particularly limited and may be appropriately selected depending on the intended purpose, but it is preferably 5 parts by mass to 25 parts by mass, more preferably 10 parts by mass to 20 parts by mass, relative to 100 parts by mass of the toner. When the amount thereof is smaller than 5 parts by mass, low temperature fixing ability, and hot offset resistance of a resulting toner may be impaired. When the amount thereof is greater than 25 parts by mass, heat resistant storage stability of the toner may be impaired, and glossiness of an image obtained after fixing and coloring ability may reduce. When the amount thereof is within the aforementioned more preferable range, it is advantageous because all of the low temperature fixing ability, hot offset resistance, and heat resistant storage stability excel.

<<Non-Crystalline Polyester Resin B>>

The non-crystalline polyester resin B preferably has a glass transition temperature of  $40^\circ\text{ C.}$  to  $80^\circ\text{ C.}$

The non-crystalline polyester resin B is preferably a linear polyester resin.

The non-crystalline polyester resin B is preferably an unmodified polyester resin. The unmodified polyester resin refers to a polyester resin that is obtained using a polyhydric alcohol and a polyvalent carboxylic acid or a derivative thereof such as a polyvalent carboxylic acid anhydride and a polyvalent carboxylic acid ester, and that is not modified with an isocyanate compound or the like. Preferably, the non-crystalline polyester resin B does not have a urethane bond or a urea bond.

The non-crystalline polyester resin B contains a dicarboxylic acid component as a constituent component, and the dicarboxylic acid component contains terephthalic acid in an amount of 50 mol % or more, which is advantageous in terms of heat resistant storage stability.

Examples of the polyhydric alcohol include diols.

Examples of the diol include adducts of bisphenol A with alkylen (C2 to C3) oxides (average addition mole number: 1 to 10) such as polyoxypropylene(2.2)-2,2-bis(4-hydroxy-phenyl)propane and polyoxyethylene(2.2)-2,2-bis(4-hydroxyphenyl)propane; ethylene glycol and propylene glycol; and hydrogenerated bisphenol A and adducts of hydrogenerated bisphenol A with alkylen (C2 to C3) oxides (average addition mole number: 1 to 10).

These may be used alone or in combination of two or more thereof.

Examples of the polyvalent carboxylic acid include dicarboxylic acids.

Examples of the dicarboxylic acid include adipic acid, phthalic acid, isophthalic acid, terephthalic acid, fumaric acid, and maleic acid; and succinic acid having, as a substituent, an alkyl group having 1 to 20 carbon atoms or an alkenyl group having 1 to 20 carbon atoms, such as dodecanyl succinic acid and octyl succinic acid.

## 16

These may be used alone or in combination of two or more thereof.

Also, in order to adjust the acid value or hydroxyl value, the non-crystalline polyester resin B may contain a trivalent or higher carboxylic acid, a trihydric or higher alcohol, or both at the end of its resin chain.

Examples of the trivalent or higher carboxylic acid include trimellitic acid, pyromellitic acid, and acid anhydrides thereof.

10 Examples of the trihydric or higher alcohol include glycerin, pentaerythritol, and trimethylpropane.

A molecular weight of the non-crystalline polyester resin B is not particularly limited and may be appropriately selected depending on the intended purpose. When the 15 molecular weight thereof is too low, the obtained toner may be poor in heat resistant storage stability and durability to stress such as stirring in a developing device. When the molecular weight thereof is too high, the obtained toner may be increased in viscoelasticity upon melting to be poor in 20 low temperature fixing ability. Hence, in GPC (gel permeation chromatography), the non-crystalline polyester resin B preferably has a weight average molecular weight (Mw) of 3,000 to 10,000, and also has a number average molecular weight (Mn) of 1,000 to 4,000. A ratio Mw/Mn is preferably 25 1.0 to 4.0.

The weight average molecular weight (Mw) of the non-crystalline polyester resin B is more preferably 4,000 to 7,000. The number average molecular weight (Mn) thereof is more preferably 1,500 to 3,000. The ratio Mw/Mn is more 30 preferably 1.0 to 3.5.

An acid value of the non-crystalline polyester resin B is not particularly limited and may be appropriately selected depending on the intended purpose, but it is preferably 1 mgKOH/g to 50 mgKOH/g, more preferably 5 mgKOH/g to 35 30 mgKOH/g. When the acid value thereof is 1 mgKOH/g or more, the obtained toner will be negatively chargeable more easily and be better in affinity to paper upon being fixed thereon, and as a result can be improved in low temperature fixing ability. When the acid value thereof is 40 more than 50 mgKOH/g, the obtained toner may be degraded in charging stability, especially charging stability to environmental changes.

The hydroxyl value of the non-crystalline polyester resin B is not particularly limited and may be appropriately 45 selected depending on the intended purpose, but it is preferably 5 mgKOH/g or more.

A glass transition temperature (Tg) of the non-crystalline polyester resin B is preferably  $40^\circ\text{ C.}$  to  $80^\circ\text{ C.}$ , more preferably  $50^\circ\text{ C.}$  to  $70^\circ\text{ C.}$  When the glass transition temperature thereof is lower than  $40^\circ\text{ C.}$ , the obtained toner may be poor in heat resistant storage stability and durability to stress such as stirring in a developing device, and also may be degraded in filming resistance. When the glass transition temperature thereof is higher than  $80^\circ\text{ C.}$ , the 55 obtained toner cannot sufficiently deform with heating and pressing upon fixing, potentially leading to insufficient low temperature fixing ability.

A molecular structure of the non-crystalline polyester resin B can be confirmed by solution-state or solid-state 60 NMR, X-ray diffraction, GC/MS, LC/MS, or IR spectroscopy. Simple methods thereof include a method for detecting, as a non-crystalline polyester resin, one that does not have absorption based on  $\delta\text{CH}$  (out-of-plane bending vibration) of olefin at  $965\text{ cm}^{-1}\pm10\text{ cm}^{-1}$  and  $990\text{ cm}^{-1}\pm10\text{ cm}^{-1}$  in an infrared absorption spectrum.

An amount of the non-crystalline polyester resin B is not particularly limited and may be appropriately selected

depending on the intended purpose, but it is preferably 50 parts by mass to 90 parts by mass relative to 100 parts by mass of the toner, more preferably 60 parts by mass to 80 parts by mass relative to 100 parts by mass of the toner. When the amount of the non-crystalline polyester resin B is less than 50 parts by mass, the pigment and the releasing agent in the toner will become degraded in dispersibility, potentially easily causing fogging on images and formation of abnormal images. When the amount of the non-crystalline polyester resin B is more than 90 parts by mass, the amounts of the crystalline polyester resin C and the non-crystalline polyester resin A will become small and hence the obtained toner may be degraded in low temperature fixing ability. The amount of the non-crystalline polyester resin B falling within the above more preferable range is advantageous since the obtained toner is excellent in all of high image quality and low temperature fixing ability.

## &lt;&lt;Crystalline Polyester Resin C&gt;&gt;

The crystalline polyester resin C exhibits thermofusion characteristics in which viscosity is drastically decreases at temperature around fixing onset temperature, as the crystalline polyester resin C has high crystallinity. By using the crystalline polyester resin C having the aforementioned characteristics together with the non-crystalline polyester resin B in the toner, the heat resistant storage stability of the toner is excellent up to the melt onset temperature owing to crystallinity, and the toner drastically decreases its viscosity (sharp melt property) at the melt onset temperature because of melting of the crystalline polyester resin C. Along with the drastic decrease in viscosity, the crystalline polyester resin C is melt together with the non-crystalline polyester resin B, to drastically decrease their viscosity to thereby be fixed. Accordingly, a toner having excellent heat resistant storage stability and low temperature fixing ability can be obtained. Moreover, the toner has excellent results in terms of a releasing width (a difference between the minimum fixing temperature and hot offset occurring temperature).

The crystalline polyester resin C is obtained from a polyhydric alcohol and a polyvalent carboxylic acid or a derivative thereof such as a polyvalent carboxylic acid anhydride and a polyvalent carboxylic acid ester.

Note that, in the present invention, the crystalline polyester resin C is one obtained from a polyhydric alcohol and a polyvalent carboxylic acid or a derivative thereof such as a polyvalent carboxylic acid anhydride and a polyvalent carboxylic acid ester, as described above, and a resin obtained by modifying a polyester resin, for example, the aforementioned prepolymer and a resin obtained through cross-link and/or chain elongation reaction of the prepolymer do not belong to the crystalline polyester resin C.

## -Polyhydric Alcohol-

The polyhydric alcohol is not particularly limited and may be appropriately selected depending on the intended purpose. Examples thereof include diol, and trihydric or higher alcohol.

Examples of the diol include saturated aliphatic diol. Examples of the saturated aliphatic diol include linear chain saturated aliphatic diol, and branched-chain saturated aliphatic diol. Among them, linear chain saturated aliphatic diol is preferable, and C2-C12 linear chain saturated aliphatic diol is more preferable. When the saturated aliphatic diol has a branched-chain structure, crystallinity of the crystalline polyester resin C may be low, which may lower the melting point. When the number of carbon atoms in the saturated aliphatic diol is greater than 12, it may be difficult to yield a material in practice. The number of carbon atoms is therefore preferably 12 or less.

Examples of the saturated aliphatic diol include ethylene glycol, 1,3-propanediol, 1,4-butanediol, 1,5-pentanediol, 1,6-hexanediol, 1,7-heptanediol, 1,8-octanediol, 1,9-nonanediol, 1,10-decanediol, 1,11-undecanediol, 1,12-dodecanediol, 1,13-tridecanediol, 1,14-tetradecanediol, 1,18-octadecanediol, and 1,14-eicosanediol. Among them, ethylene glycol, 1,4-butanediol, 1,6-hexanediol, 1,8-octanediol, 1,10-decanediol, and 1,12-dodecanediol are preferable, as they give high crystallinity to a resulting crystalline polyester resin, and give excellent sharp melt properties.

Examples of the trihydric or higher alcohol include glycerin, trimethylol ethane, trimethylolpropane, and pentaerythritol.

These may be used alone or in combination of two or more thereof.

## -Polyvalent Carboxylic Acid-

The polyvalent carboxylic acid is not particularly limited and may be appropriately selected depending on the intended purpose. Examples thereof include divalent carboxylic acid, and trivalent or higher carboxylic acid.

Examples of the divalent carboxylic acid include: saturated aliphatic dicarboxylic acid, such as oxalic acid, succinic acid, glutaric acid, adipic acid, suberic acid, azelaic acid, sebacic acid, 1,9-nonanedicarboxylic acid, 1,10-decanedicarboxylic acid, 1,12-dodecanedicarboxylic acid, 1,14-tetradecanedicarboxylic acid, and 1,18-octadecanedicarboxylic acid; aromatic dicarboxylic acid of dibasic acid, such as phthalic acid, isophthalic acid, terephthalic acid, naphthalene-2,6-dicarboxylic acid, malonic acid, and mesaconic acid; and anhydrides of the foregoing compounds, and lower (C1-C3) alkyl ester of the foregoing compounds.

Examples of the trivalent or higher carboxylic acid include 1,2,4-benzenetricarboxylic acid, 1,2,5-benzenetricarboxylic acid, 1,2,4-naphthalene tricarboxylic acid, anhydrides thereof, and lower (C1-C3) alkyl esters thereof.

Moreover, the polyvalent carboxylic acid may contain, other than the saturated aliphatic dicarboxylic acid or aromatic dicarboxylic acid, dicarboxylic acid containing a sulfonic acid group. Further, the polyvalent carboxylic acid may contain, other than the saturated aliphatic dicarboxylic acid or aromatic dicarboxylic acid, dicarboxylic acid having a double bond.

These may be used alone or in combination of two or more thereof.

The crystalline polyester resin C is preferably composed of a linear chain saturated aliphatic dicarboxylic acid having 4 to 12 carbon atoms and a linear chain saturated aliphatic diol having 2 to 12 carbon atoms. Specifically, the crystalline polyester resin C preferably contains a constituent unit derived from a saturated aliphatic dicarboxylic acid having 4 to 12 carbon atoms, and a constituent unit derived from a saturated aliphatic diol having 2 to 12 carbon atoms. As a result of this, crystallinity increases, and sharp melt properties improve, and therefore it is preferable as excellent low temperature fixing ability of the toner is exhibited.

A melting point of the crystalline polyester resin C is not particularly limited and may be appropriately selected depending on the intended purpose, but it is preferably 60° C. to 80° C. When the melting point thereof is lower than 60° C., the crystalline polyester resin tends to be melted at low temperature, which may impair heat resistant storage stability of the toner. When the melting point thereof is higher than 80° C., melting of the crystalline polyester resin C with heat applied during fixing may be insufficient, which may impair low temperature fixing ability of the toner.

A molecular weight of the crystalline polyester resin C is not particularly limited and may be appropriately selected

depending on the intended purpose. Since those having a sharp molecular weight distribution and low molecular weight have excellent low temperature fixing ability, and heat resistant storage stability of a resulting toner lowers as an amount of a low molecular weight component, an o-dichlorobenzene soluble component of the crystalline polyester resin C preferably has the weight average molecular weight (Mw) of 3,000 to 30,000, number average molecular weight (Mn) of 1,000 to 10,000, and Mw/Mn of 1.0 to 10, as measured by GPC.

Further, it is more preferred that the weight average molecular weight (Mw) thereof be 5,000 to 15,000, the number average molecular weight (Mn) there be 2,000 to 10,000, and the Mw/Mn be 1.0 to 5.0.

An acid value of the crystalline polyester resin C is not particularly limited and may be appropriately selected depending on the intended purpose, but it is preferably 5 mgKOH/g or higher, more preferably 10 mgKOH/g or higher for achieving the desired low temperature fixing ability in view of affinity between paper and the resin. Meanwhile, the acid value thereof is preferably 45 mgKOH/g or lower for the purpose of improving hot offset resistance.

A hydroxyl value of the crystalline polyester resin C is not particularly limited and may be appropriately selected depending on the intended purpose, but it is preferably 0 mgKOH/g to 50 mgKOH/g, more preferably 5 mgKOH/g to 50 mgKOH/g, for achieving the desired low temperature fixing ability and excellent charging properties.

A molecular structure of the crystalline polyester resin C can be confirmed by solution-state or solid-state NMR, X-ray diffraction, GC/MS, LC/MS, or IR spectroscopy. Simple methods thereof include a method for detecting, as the crystalline polyester resin C, one that has absorption based on SCH (out-of-plane bending vibration) of olefin at  $965\text{ cm}^{-1}\pm10\text{ cm}^{-1}$  and  $990\text{ cm}^{-1}\pm10\text{ cm}^{-1}$  in an infrared absorption spectrum.

An amount of the crystalline polyester resin C is not particularly limited and may be appropriately selected depending on the intended purpose, but it is preferably 3 parts by mass to 20 parts by mass, more preferably 5 parts by mass to 15 parts by mass, relative to 100 parts by mass of the toner. When the amount thereof is smaller than 3 parts by mass, the crystalline polyester resin C does not give sufficient sharp melt properties, which may lead to insufficient low temperature fixing ability of a resulting toner. When the amount thereof is greater than 20 parts by mass, a resulting toner may have low heat resistant storage stability, and tends to cause fogging of an image. When the amount thereof is within the aforementioned more preferable range, it is advantageous because a resulting toner is excellent in terms of both high image quality and low temperature fixing ability.

#### <Other Components>

Examples of other components include a releasing agent, colorant, charge controlling agent, external additive, a flow improving agent, a cleaning improving agent, and a magnetic material.

#### -Releasing Agent-

The releasing agent is appropriately selected from those known in the art without any limitation.

Examples of wax serving as the releasing agent include: natural wax, such as vegetable wax (e.g., carnauba wax, cotton wax, Japan wax and rice wax), animal wax (e.g., bees wax and lanolin), mineral wax (e.g., ozokerite and ceresine) and petroleum wax (e.g., paraffin wax, microcrystalline wax and petrolatum).

Examples of the wax other than the above natural wax include synthetic hydrocarbon wax (e.g., Fischer-Tropsch wax and polyethylene wax; and synthetic wax (e.g., ester wax, ketone wax and ether wax).

Further, other examples of the releasing agent include fatty acid amides such as 12-hydroxystearic acid amide, stearic amide, phthalic anhydride imide and chlorinated hydrocarbons; low-molecular-weight crystalline polymers such as acrylic homopolymers (e.g., poly-n-stearyl methacrylate and poly-n-lauryl methacrylate) and acrylic copolymers (e.g., n-stearyl acrylate-ethyl methacrylate copolymers); and crystalline polymers having a long alkyl group as a side chain.

Among them, hydrocarbon wax, such as paraffin wax, microcrystalline wax, Fischer-Tropsch wax, polyethylene wax, and polypropylene wax, is preferable.

A melting point of the releasing agent is not particularly limited and may be appropriately selected depending on the intended purpose, but it is preferably 60° C. to 80° C. When the melting point thereof is lower than 60° C., the releasing agent tends to melt at low temperature, which may impair heat resistant storage stability. When the melting point thereof is higher than 80° C., the releasing agent is not sufficiently melted to thereby cause fixing offset even in the case where the resin is melted and is in the fixing temperature range, which may cause defects in an image.

An amount of the releasing agent is appropriately selected depending on the intended purpose without any limitation, but it is preferably 2 parts by mass to 10 parts by mass, more preferably 3 parts by mass to 8 parts by mass, relative to 100 parts by mass of the toner. When the amount thereof is smaller than 2 parts by mass, a resulting toner may have insufficient hot offset resistance, and low temperature fixing ability during fixing. When the amount thereof is greater than 10 parts by mass, a resulting toner may have insufficient heat resistant storage stability, and tends to cause fogging in an image. When the amount thereof is within the aforementioned more preferable range, it is advantageous because image quality and fixing stability can be improved.

#### -Colorant-

The colorant is appropriately selected depending on the intended purpose without any limitation, and examples thereof include carbon black, a nigrosin dye, iron black, naphthol yellow S, Hansa yellow (10G, 5G and G), cadmium yellow, yellow iron oxide, yellow ochre, yellow lead, titanium yellow, polyazo yellow, oil yellow, Hansa yellow (GR, A, RN and R), pigment yellow L, benzidine yellow (G and GR), permanent yellow (NCG), vulcan fast yellow (5G, R), tartrazin lake, quinoline yellow lake, anthrason yellow BGL, isoindolinon yellow, colcothar, red lead, lead vermillion, cadmium red, cadmium mercury red, antimony vermillion, permanent red 4R, parared, fiser red, parachloroorthonitro anilin red, lithol fast scarlet G, brilliant fast scarlet, brilliant carmine BS, permanent red (F2R, F4R, FRL, FRL and F4RH), fast scarlet VD, vulcan fast rubin B, brilliant scarlet G, lithol rubin GX, permanent red F5R, brilliant carmine 6B, pigment scarlet 3B, Bordeaux 5B, toluidine Maroon, permanent Bordeaux F2K, Helio Bordeaux BL, Bordeaux 10B, BON maroon light, BON maroon medium, eosin lake, rhodamine lake B, rhodamine lake Y, alizarin lake, thioindigo red B, thioindigo maroon, oil red, quinacridone red, pyrazolone red, polyazo red, chrome vermillion, benzidine orange, perinone orange, oil orange, cobalt blue, cerulean blue, alkali blue lake, peacock blue lake, Victoria blue lake, metal-free phthalocyanine blue, phthalocyanine blue, fast sky blue, indanthrene blue (RS and BC), indigo, ultramarine, iron blue, anthraquinone blue, fast violet B,

methyl violet lake, cobalt purple, manganese violet, dioxane violet, anthraquinone violet, chrome green, zinc green, chromium oxide, viridian, emerald green, pigment green B, naphthol green B, green gold, acid green lake, malachite green lake, phthalocyanine green, anthraquinone green, titanium oxide, zinc flower, and lithopone.

An amount of the colorant is not particularly limited and may be appropriately selected depending on the intended purpose, but it is preferably 1 part by mass to 15 parts by mass, more preferably 3 parts by mass to 10 parts by mass, relative to 100 parts by mass of the toner.

The colorant may be used as a master batch in which the colorant forms a composite with a resin. Examples of the binder resin kneaded in the production of, or together with the master batch include, other than the aforementioned non-crystalline polyester resin, polymer of styrene or substitution thereof (e.g., polystyrene, poly-p-chlorostyrene, and polyvinyl); styrene copolymer (e.g., styrene-p-chlorostyrene copolymer, styrene-propylene copolymer, styrene-vinyl toluene copolymer, styrene-vinyl naphthalene copolymer, styrene-methyl acrylate copolymer, styrene-ethyl acrylate copolymer, styrene-butyl acrylate copolymer, styrene-octyl acrylate copolymer, styrene-methyl methacrylate copolymer, styrene-ethyl methacrylate copolymer, styrene-butyl methacrylate copolymer, styrene-methyl  $\alpha$ -chloromethacrylate copolymer, styrene-acrylonitrile copolymer, styrene-vinyl methyl ketone copolymer, styrene-butadiene copolymer, styrene-isoprene copolymer, styrene-acrylonitrile-indene copolymer, styrene-maleic acid copolymer, and styrene-maleic acid ester copolymer); and others including polymethyl methacrylate, polybutyl methacrylate, polyvinyl chloride, polyvinyl acetate, polyethylene, polypropylene, polyester, epoxy resin, epoxy polyol resin, polyurethane, polyamide, polyvinyl butyral, polyacrylic acid resin, rosin, modified rosin, a terpene resin, an aliphatic or alicyclic hydrocarbon resin, an aromatic petroleum resin, chlorinated paraffin, and paraffin wax. These may be used independently, or in combination.

The master batch can be prepared by mixing and kneading the colorant with the resin for the master batch. In the mixing and kneading, an organic solvent may be used for improving the interactions between the colorant and the resin. Moreover, the master batch can be prepared by a flashing method in which an aqueous paste containing a colorant is mixed and kneaded with a resin and an organic solvent, and then the colorant is transferred to the resin to remove the water and the organic solvent. This method is preferably used because a wet cake of the colorant is used as it is, and it is not necessary to dry the wet cake of the colorant to prepare a colorant. In the mixing and kneading of the colorant and the resin, a high-shearing disperser (e.g., a three-roll mill) is preferably used.

#### -Charge Controlling Agent-

The charge controlling agent is appropriately selected depending on the intended purpose without any limitation, and examples thereof include nigrosine dyes, triphenylmethane dyes, chrome-containing metal complex dyes, molybdcic acid chelate pigments, rhodamine dyes, alkoxy amines, quaternary ammonium salts (including fluorine-modified quaternary ammonium salts), alkylamides, phosphorus, phosphorus compounds, tungsten, tungsten compounds, fluorine active agents, metal salts of salicylic acid, and metal salts of salicylic acid derivatives.

Specific examples thereof include: nigrosine aye BONTRON 03, quaternary ammonium salt BONTRON P-51, metal-containing azo dye BONTRON S-34, oxynaphthoic acid-based metal complex E-82, salicylic acid-based metal

complex E-84 and phenol condensate E-89 (all manufactured by ORIENT CHEMICAL INDUSTRIES CO., LTD); quaternary ammonium salt molybdenum complex TP-302 and TP-415 (all manufactured by Hodogaya Chemical Co., Ltd.); LRA-901; boron complex LR-147 (manufactured by Japan Carlit Co., Ltd.); copper phthalocyanine; perylene; quinacridone; azo pigments; and polymeric compounds having, as a functional group, a sulfonic acid group, carboxyl group, quaternary ammonium salt, etc.

An amount of the charge controlling agent is not particularly limited and may be appropriately selected depending on the intended purpose, but it is preferably 0.1 parts by mass to 10 parts by mass, more preferably 0.2 parts by mass to 5 parts by mass, relative to 100 parts by mass of the toner. When the amount thereof is greater than 10 parts by mass, the charging ability of the toner becomes excessive, which may reduce the effect of the charge controlling agent, increase electrostatic force to a developing roller, leading to low flowability of the developer, or low image density of the resulting image. These charge controlling agents may be dissolved and dispersed after being melted and kneaded together with the master batch, and/or resin. The charge controlling agents can be, of course, directly added to an organic solvent when dissolution and dispersion is performed. Alternatively, the charge controlling agents may be fixed on surfaces of toner particles after the production of the toner particles.

#### -External Additive-

As for the external additive, other than oxide particles, a combination of inorganic particles and hydrophobic-treated inorganic particles can be used. The average primary particle diameter of the hydrophobic-treated particles is preferably 1 nm to 100 nm. More preferred are 5 nm to 70 nm of the inorganic particles.

Moreover, it is preferred that the external additive contain at least one type of hydrophobic-treated inorganic particles having the average primary particle diameter of 20 nm or smaller, and at least one type of inorganic particles having the average primary particle diameter of 30 nm or greater. Moreover, the external additive preferably has the BET specific surface area of 20 m<sup>2</sup>/g to 500 m<sup>2</sup>/g.

The external additive is not particularly limited and may be appropriately selected depending on the intended purpose. Examples thereof include silica particles, hydrophobic silica, fatty acid metal salts (e.g., zinc stearate, and aluminum stearate), metal oxide (e.g., titania, alumina, tin oxide, and antimony oxide), and a fluoropolymer.

Examples of the suitable additive include hydrophobic silica, titania, titanium oxide, and alumina particles. Examples of the silica particles include R972, R974, RX200, RY200, R202, R805, and R812 (all manufactured by Nippon Aerosil Co., Ltd.). Examples of the titania particles include P-25 (manufactured by Nippon Aerosil Co., Ltd.); STT-30, STT-65C-S (both manufactured by Titan Kogyo, Ltd.); TAF-140 (manufactured by Fuji Titanium Industry Co., Ltd.); and MT-150W, MT-500B, MT-600B, MT-150A (all manufactured by TAYCA CORPORATION).

Examples of the hydrophobic treated titanium oxide particles include: T-805 (manufactured by Nippon Aerosil Co., Ltd.); STT-30A, STT-65S-S (both manufactured by Titan Kogyo, Ltd.); TAF-500T, TAF-1500T (both manufactured by Fuji Titanium Industry Co., Ltd.); MT-100S, MT-100T (both manufactured by TAYCA CORPORATION); and IT-S (manufactured by ISHIHARA SANGYO KAISHA, LTD.).

The hydrophobic-treated oxide particles, hydrophobic-treated silica particles, hydrophobic-treated titania particles, and hydrophobic-treated alumina particles are obtained, for

example, by treating hydrophilic particles with a silane coupling agent, such as methyltrimethoxy silane, methyltriethoxy silane, and octyltrimethoxy silane. Moreover, silicone oil-treated oxide particles, or silicone oil-treated inorganic particles, which have been treated by adding silicone oil optionally with heat, are also suitably used as the external additive.

Examples of the silicone oil include dimethyl silicone oil, methylphenyl silicone oil, chlorophenyl silicone oil, methyl hydrogen silicone oil, alkyl-modified silicone oil, fluorine-modified silicone oil, polyether-modified silicone oil, alcohol-modified silicone oil, amino-modified silicone oil, epoxy-modified silicone oil, epoxy-polyether-modified silicone oil, phenol-modified silicone oil, carboxyl-modified silicone oil, mercapto-modified silicone oil, methacryl-modified silicone oil, and  $\alpha$ -methylstyrene-modified silicone oil.

Examples of the inorganic particles include silica, alumina, titanium oxide, barium titanate, magnesium titanate, calcium titanate, strontium titanate, iron oxide, copper oxide, zinc oxide, tin oxide, quartz sand, clay, mica, wollastonite, diatomaceous earth, chromic oxide, cerium oxide, red iron oxide, antimony trioxide, magnesium oxide, zirconium oxide, barium sulfate, barium carbonate, calcium carbonate, silicon carbide, and silicon nitride. Among them, silica and titanium dioxide are preferable.

An amount of the external additive is not particularly limited and may be appropriately selected depending on the intended purpose, but it is preferably 0.1 parts by mass to 5 parts by mass, more preferably 0.3 parts by mass to 3 parts by mass, relative to 100 parts by mass of the toner.

The average particle diameter of primary particles of the inorganic particles is not particularly limited and may be appropriately selected depending on the intended purpose, but it is preferably 100 nm or smaller, more preferably 3 nm to 70 nm. When it is smaller than the aforementioned range, the inorganic particles are embedded in the toner particles, and therefore the function of the inorganic particles may not be effectively exhibited. When the average particle diameter thereof is greater than the aforementioned range, the inorganic particles may unevenly damage a surface of a photoconductor, and hence not preferable.

#### -Flowability Improving Agent-

The flowability improving agent is not particularly limited and may be appropriately selected depending on the intended purpose so long as it is capable of performing surface treatment of the toner to increase hydrophobicity, and preventing degradations of flow properties and charging properties of the toner even in a high humidity environment. Examples thereof include a silane-coupling agent, a sililation agent, a silane-coupling agent containing a fluoroalkyl group, an organic titanate-based coupling agent, an aluminum-based coupling agent, silicone oil, and modified silicone oil. It is particularly preferred that the silica or titanium oxide be used as hydrophobic silica or hydrophobic titanium oxide treated with the aforementioned flow improving agent.

#### -Cleanability Improving Agent-

The cleanability improving agent is not particularly limited and may be appropriately selected depending on the intended purpose so long as it can be added to the toner for the purpose of removing the developer remained on a photoconductor or primary transfer member after transferring. Examples thereof include: fatty acid metal salt such as zinc stearate, calcium stearate, and stearic acid; and polymer particles produced by soap-free emulsion polymerization, such as polymethyl methacrylate particles, and polystyrene particles. The polymer particles are preferably those having

a relatively narrow particle size distribution, and the polymer particles having the volume average particle diameter of 0.01  $\mu\text{m}$  to 1  $\mu\text{m}$  are preferably used.

#### -Magnetic Material-

The magnetic material is not particularly limited and may be appropriately selected depending on the intended purpose. Examples thereof include iron powder, magnetite, and ferrite. Among them, a white magnetic material is preferable in terms of a color tone.

#### 10 <<Method for Measuring Particle Size Distribution>>

The volume average particle diameter (D4) and number average particle diameter (Dn) of the toner and the ratio thereof (D4/Dn) can be measured, for example, by means of Coulter Counter TA-II or Coulter Multisizer II (both products are of Beckman Coulter, Inc.). In the present invention, Coulter Multisizer II was used. The measurement method will be explained below.

First, 0.1 mL to 5 mL of a surfactant (preferably alkyl benzene sulfonate (nonionic surfactant)) was added as a dispersant to 100 mL to 150 mL of an electrolyte. Note that, the electrolyte is an about 1% by mass aqueous solution prepared by using a primary sodium chloride, and for example, ISOTON-II (of Beckman Coulter, Inc.) is used as the electrolyte. Next, to the resulting mixture, 2 mg to 20 mg of a sample is added and suspended, and the mixture is dispersed by means of an ultrasonic wave disperser for about 1 minute to about 3 minutes. The volume and number of the toner particles or toner are measured from the obtained dispersion liquid using the aforementioned measuring device with an aperture of 100  $\mu\text{m}$ , and then the volume distribution and number distribution of the toner are calculated. From the obtained distributions, the volume average particle diameter (D4), and number average particle diameter (Dn) of the toner can be determined.

35 Note that, as a channel, the following 13 channels are used: 2.00  $\mu\text{m}$  or larger, but smaller than 2.52  $\mu\text{m}$ ; 2.52  $\mu\text{m}$  or larger, but smaller than 3.17  $\mu\text{m}$ ; 3.17  $\mu\text{m}$  or larger, but smaller than 4.00  $\mu\text{m}$ ; 4.00  $\mu\text{m}$  or larger, but smaller than 5.04  $\mu\text{m}$ ; 5.04  $\mu\text{m}$  or larger, but smaller than 6.35  $\mu\text{m}$ ; 6.35  $\mu\text{m}$  or larger, but smaller than 8.00  $\mu\text{m}$ ; 8.00  $\mu\text{m}$  or larger, but smaller than 10.08  $\mu\text{m}$ ; 10.08  $\mu\text{m}$  or larger, but smaller than 12.70  $\mu\text{m}$ ; 12.70  $\mu\text{m}$  or larger, but smaller than 16.00  $\mu\text{m}$ ; 16.00  $\mu\text{m}$  or larger, but smaller than 20.20  $\mu\text{m}$ ; 20.20  $\mu\text{m}$  or larger, but smaller than 25.40  $\mu\text{m}$ ; 25.40  $\mu\text{m}$  or larger, but smaller than 32.00  $\mu\text{m}$ ; and 32.00  $\mu\text{m}$  or larger, but smaller than 40.30  $\mu\text{m}$ . The target particles for the measurement are particles having the diameters of 2.00  $\mu\text{m}$  or larger, but smaller than 40.30  $\mu\text{m}$ .

#### 30 <<Measurement of Molecular Weight>>

45 A molecular weight of each constituent component of a toner can be measured, for example, by the following method.

50 Gel permeation chromatography (GPC) measuring device: GPC-8220GPC (manufactured by TOSOH CORPORATION)

55 Column: TSKgel SuperHZM-H 15 cm, three connected columns (manufactured by TOSOH CORPORATION)

Temperature: 40° C.

Solvent: THF

Flow rate: 0.35 mL/min

60 Sample: 100  $\mu\text{L}$  of a 0.15% by mass sample to be supplied

65 As for the pretreatment of the sample, the sample is dissolved in tetrahydrofuran (THF) (containing a stabilizer, manufactured by Wako Chemical Industries, Ltd.) to give a concentration of 0.15% by mass, the resulting solution is then filtered through a filter having a pore size of 0.2  $\mu\text{m}$ , and the filtrate from the filtration is used as a sample. The

measurement is performed by supplying 100  $\mu\text{L}$  of the tetrahydrofuran (THF) sample solution.

For the measurement of the molecular weight of the sample, a molecular weight distribution of the sample is calculated from the relationship between the logarithmic value of the calibration curve prepared from a several monodispersible polystyrene standard samples and the number of counts. As the standard polystyrene samples for preparing the calibration curve, Showdex STANDARD Std. Nos. S-7300, S-210, S-390, S-875, S-1980, S-10.9, S-629, S-3.0, and S-0.580 of SHOWA DENKO K.K., and toluene are used. As the detector, a refractive index (RI) detector is used.

<Production Method of Toner>

A production method of the toner is not particularly limited and may be appropriately selected depending on the intended purpose, but the toner is preferably granulated by dispersing, in an aqueous medium, an oil phase containing the polyester resin, and if necessary, further containing the releasing agent and the colorant.

Also, the toner is more preferably granulated by dispersing, in an aqueous medium, an oil phase containing: as the non-crystalline polyester resin, a polyester resin which is a prepolymer containing a urethane bond, a urea bond, or both; and a polyester resin not containing a urethane bond, a urea bond, or both; preferably further containing the crystalline polyester resin; and if necessary, further containing the releasing agent, the colorant, etc.

As one example of such a production method of the toner, a conventionally dissolution suspension method is listed. As one example of the production method of the toner, a method for forming toner base particles while extending the non-crystalline polyester resin through a chain-elongation reaction and/or cross-link reaction between the prepolymer and the curing agent will be described hereinafter. In such a method, a preparation of an aqueous medium, preparation of an oil phase containing a toner material, emulsification and/or dispersion of the toner material, and removal of an organic solvent are carried out.

-Preparation of Aqueous Medium (Aqueous Phase)-

The preparation of the aqueous phase can be carried out, for example, by dispersing resin particles in an aqueous medium. An amount of the resin particles in the aqueous medium is not particularly limited and may be appropriately selected depending on the intended purpose, but it is preferably 0.5 parts by mass to 10 parts by mass relative to 100 parts by mass of the aqueous medium.

The aqueous medium is not particularly limited and may be appropriately selected depending on the intended purpose. Examples thereof include water, a solvent miscible with water, and a mixture thereof. These may be used independently, or in combination. Among them, water is preferable.

The solvent miscible with water is not particularly limited and may be appropriately selected depending on the intended purpose. Examples thereof include alcohol, dimethyl formamide, tetrahydrofuran, cellosolve, and lower ketone. The alcohol is not particularly limited and may be appropriately selected depending on the intended purpose. Examples thereof include methanol, isopropanol, and ethylene glycol. The lower ketone is not particularly limited and may be appropriately selected depending on the intended purpose. Examples thereof include acetone and methyl ethyl ketone.

-Preparation of Oil Phase-

The oil phase containing the toner materials can be prepared by dissolving or dispersing, in an organic solvent,

toner materials containing: at least a polyester resin which is a prepolymer containing a urethane bond, a urea bond, or both; a polyester resin not containing a urethane bond, a urea bond, or both; and the crystalline polyester resin, and if necessary, further containing the curing agent, the releasing agent, the colorant, etc.

The organic solvent is not particularly limited and may be appropriately selected depending on the intended purpose, but it is preferably an organic solvent having a boiling point of lower than 150° C., as removal thereof is easy.

The organic solvent having the boiling point of lower than 150° C. is not particularly limited and may be appropriately selected depending on the intended purpose. Examples thereof include toluene, xylene, benzene, carbon tetrachloride, methylene chloride, 1,2-dichloroethane, 1,1,2-trichloroethane, trichloroethylene, chloroform, monochlorobenzene, dichloroethylidene, methyl acetate, ethyl acetate, methyl ethyl ketone, and methyl isobutyl ketone. These may be used alone or in combination of two or more thereof.

Among them, ethyl acetate, toluene, xylene, benzene, methylene chloride, 1,2-dichloroethane, chloroform, and carbon tetrachloride are particularly preferable, and ethyl acetate is more preferable.

-Emulsification or Dispersion-

The emulsification or dispersion of the toner materials can be carried out by dispersing the oil phase containing the toner materials in the aqueous medium. In the course of the emulsification or dispersion of the toner material, the curing agent and the prepolymer are allowed to carry out a chain-elongation reaction or cross-link reaction.

The reaction conditions (e.g., the reaction time and reaction temperature) for generating the prepolymer are not particularly limited and may be appropriately selected depending on a combination of the curing agent and the prepolymer.

The reaction time is not particularly limited and may be appropriately selected depending on the intended purpose, but it is preferably 10 minutes to 40 hours, more preferably 2 hours to 24 hours.

The reaction temperature is not particularly limited and may be appropriately selected depending on the intended purpose, but it is preferably 0° C. to 150° C., more preferably 40° C. to 98° C.

A method for stably forming a dispersion liquid in the aqueous medium is not particularly limited and may be appropriately selected depending on the intended purpose. Examples thereof include a method in which an oil phase, which has been prepared by dissolving and/or dispersing a toner material in a solvent, is added to a phase of an aqueous medium, followed by dispersing with shear force.

A disperser used for the dispersing is not particularly limited and may be appropriately selected depending on the intended purpose. Examples thereof include a low-speed shearing disperser, a high-speed shearing disperser, a friction disperser, a high-pressure jetting disperser and an ultrasonic wave disperser.

Among them, the high-speed shearing disperser is preferable, because it can control the particle diameters of the dispersed elements (oil droplets) to the range of 2  $\mu\text{m}$  to 20  $\mu\text{m}$ .

In the case where the high-speed shearing disperser is used, the conditions for dispersing, such as the rotating speed, dispersion time, and dispersion temperature, may be appropriately selected depending on the intended purpose.

The rotational speed is not particularly limited and may be appropriately selected depending on the intended purpose,

but it is preferably 1,000 rpm to 30,000 rpm, more preferably 5,000 rpm to 20,000 rpm.

The dispersion time is not particularly limited and may be appropriately selected depending on the intended purpose, but it is preferably 0.1 minutes to 5 minutes in case of a batch system.

The dispersion temperature is not particularly limited and may be appropriately selected depending on the intended purpose, but it is preferably 0° C. to 150° C., more preferably 40° C. to 98° C. under pressure. Note that, generally speaking, dispersion can be easily carried out, as the dispersion temperature is higher.

An amount of the aqueous medium used for the emulsification or dispersion of the toner material is not particularly limited and may be appropriately selected depending on the intended purpose, but it is preferably 50 parts by mass to 2,000 parts by mass, more preferably 100 parts by mass to 1,000 parts by mass, relative to 100 parts by mass of the toner material.

When the amount of the aqueous medium is smaller than 50 parts by mass, the dispersion state of the toner material is impaired, which may result a failure in attaining toner base particles having desired particle diameters. When the amount thereof is greater than 2,000 parts by mass, the production cost may increase.

When the oil phase containing the toner material is emulsified or dispersed, a dispersant is preferably used for the purpose of stabilizing dispersed elements, such as oil droplets, and gives a shape particle size distribution as well as giving desirable shapes of toner particles.

The dispersant is not particularly limited and may be appropriately selected depending on the intended purpose. Examples thereof include a surfactant, a water-insoluble inorganic compound dispersant, and a polymer protective colloid. These may be used alone or in combination of two or more thereof. Among them, the surfactant is preferable.

The surfactant is not particularly limited and may be appropriately selected depending on the intended purpose. Examples thereof include an anionic surfactant, a cationic surfactant, a nonionic surfactant, and an amphoteric surfactant.

The anionic surfactant is not particularly limited and may be appropriately selected depending on the intended purpose. Examples thereof include alkyl benzene sulfonic acid salts,  $\alpha$ -olefin sulfonic acid salts and phosphoric acid esters. Among them, those having a fluoroalkyl group are preferable.

#### -Removal of Organic Solvent-

A method for removing the organic solvent from the dispersion liquid such as the emulsified slurry is not particularly limited and may be appropriately selected depending on the intended purpose. Examples thereof include: a method in which an entire reaction system is gradually heated to evaporate out the organic solvent in the oil droplets; and a method in which the dispersion liquid is sprayed in a dry atmosphere to remove the organic solvent in the oil droplets.

As the organic solvent removed, toner base particles are formed. The toner base particles can be subjected to washing and drying, and can be further subjected to classification. The classification may be carried out in a liquid by removing small particles by cyclone, a decanter, or centrifugal separator, or may be performed on particles after drying.

The obtained toner base particles may be mixed with particles such as the external additive, and the charge controlling agent. By applying a mechanical impact during

the mixing, the particles such as the external additive can be prevented from fall off from surfaces of the toner base particles.

A method for applying the mechanical impact is not particularly limited and may be appropriately selected depending on the intended purpose. Examples thereof include: a method for applying impulse force to a mixture by a blade rotating at high speed; a method for adding a mixture into a high-speed air flow and accelerating the speed of the flow to thereby make the particles crash into other particles, or make the composite particles crush into an appropriate impact board.

A device used for this method is appropriately selected depending on the intended purpose without any limitation, and examples thereof include ANGMILL (product of Hosokawa Micron Corporation), an apparatus produced by modifying I-type mill (product of Nippon Pneumatic Mfg. Co., Ltd.) to reduce the pulverizing air pressure, a hybridization system (product of Nara Machinery Co., Ltd.), a krypton system (product of Kawasaki Heavy Industries, Ltd.) and an automatic mortar. (Developer)

A developer of the present invention contains at least the toner, and may further contain appropriately selected other components, such as carrier, if necessary.

Accordingly, the developer has excellent transfer properties, and charging ability, and can stably form high quality images. Note that, the developer may be a one-component developer, or a two-component developer, but it is preferably a two-component developer when it is used in a high speed printer corresponding to recent high information processing speed, because the service life thereof can be improved.

In the case where the developer is used as a one-component developer, the diameters of the toner particles do not vary largely even when the toner is supplied and consumed repeatedly, the toner does not cause filming to a developing roller, nor fuse to a layer thickness regulating member such as a blade for thinning a thickness of a layer of the toner, and provides excellent and stable developing ability and image even when it is stirred in the developing device over a long period of time.

In the case where the developer is used as a two-component developer, the diameters of the toner particles in the developer do not vary largely even when the toner is supplied and consumed repeatedly, and the toner can provide excellent and stable developing ability even when the toner is stirred in the developing device over a long period of time.

#### <Carrier>

The carrier is appropriately selected depending on the intended purpose without any limitation, but it is preferably a carrier containing a core, and a resin layer covering the core.

#### -Core-

A material of the core is appropriately selected depending on the intended purpose without any limitation, and examples thereof include a 50 emu/g to 90 emu/g manganese-strontium (Mn—Sr) material, and a 50 emu/g to 90 emu/g manganese-magnesium (Mn—Mg) material. To secure a sufficient image density, use of a hard magnetic material such as iron powder (100 emu/g or higher), and magnetite (75 emu/g to 120 emu/g) is preferable. Moreover, use of a soft magnetic material such as a 30 emu/g to 80 emu/g copper-zinc material is preferable because an impact applied to a photoconductor by the developer born on a bearing member in the form of a brush can be reduced, which is an advantageous for improving image quality.

These may be used alone or in combination of two or more thereof.

The volume average particle diameter of the core is not particularly limited and may be appropriately selected depending on the intended purpose, but it is preferably 10  $\mu\text{m}$  to 150  $\mu\text{m}$ , more preferably 40  $\mu\text{m}$  to 100  $\mu\text{m}$ . When the volume average particle diameter thereof is smaller than 10  $\mu\text{m}$ , the proportion of fine particles in the distribution of carrier particle diameters increases, causing carrier scattering because of low magnetization per carrier particle. When the volume average particle diameter thereof is greater than 150  $\mu\text{m}$ , the specific surface area reduces, which may cause toner scattering, causing reproducibility especially in a solid image portion in a full color printing containing many solid image portions.

In the case where the toner is used for a two-component developer, the toner is used by mixing with the carrier. An amount of the carrier in the two-component developer is not particularly limited and may be appropriately selected depending on the intended purpose, but it is preferably 90 parts by mass to 98 parts by mass, more preferably 93 parts by mass to 97 parts by mass, relative to 100 parts by mass of the two-component developer.

The developer of the present invention may be suitably used in image formation by various known electrophotographies such as a magnetic one-component developing method, a non-magnetic one-component developing method, and a two-component developing method.

(Developer Accommodating Container)

A developer accommodating container of the present invention accommodates the developer of the present invention. The container thereof is not particularly limited and may be appropriately selected from known containers. Examples thereof include those having a cap and a container main body.

The size, shape, structure and material of the container main body are not particularly limited. The container main body preferably has, for example, a hollow-cylindrical shape. Particularly preferably, it is a hollow-cylindrical body whose inner surface has spirally-arranged concavo-convex portions some or all of which can be transferred to an outlet port through rotation. The material for the developer-accommodating container is not particularly limited and is preferably those from which the container main body can be formed with high dimensional accuracy. Examples thereof include polyester resins, polyethylene resins, polypropylene resins, polystyrene resins, polyvinyl chloride resins, polyacrylic acids, polycarbonate resins, ABS resins and polyacetal resins.

The above developer accommodating container has excellent handleability; i.e., is suitable for storage, transportation, and is suitably used for supply of the developer with being detachably mounted to, for example, the below-described process cartridge and image forming apparatus.

(Image Forming Apparatus and Image Forming Method)

An image forming apparatus of the present invention includes at least an electrostatic latent image bearing member, an electrostatic latent image forming unit, and a developing unit, and if necessary, further includes other units.

An image forming method of the present invention includes at least an electrostatic latent image forming step and a developing step, and if necessary, further includes other steps.

The image forming method can suitably be performed by the image forming apparatus, the electrostatic latent image forming step can suitably be performed by the electrostatic

latent image forming unit, the developing step can suitably be performed by the developing unit, and the other steps can suitably be performed by the other units.

<Electrostatic Latent Image Bearing Member>

5 The material, structure, and size of the electrostatic latent image bearing member are not particularly limited and may be appropriately selected from those known in the art. Regarding the material, the electrostatic latent image bearing member is, for example, an inorganic photoconductor 10 made of amorphous silicon or selenium, or an organic photoconductor made of polysilane or phthalopolymethine. Among them, an amorphous silicon photoconductor is preferred since it has a long service life.

The amorphous silicon photoconductor may be, for 15 example, a photoconductor having a support and an electrically photoconductive layer of a-Si, which is formed on the support heated to 50° C. to 400° C. with a film forming method such as vacuum vapor deposition, sputtering, ion plating, thermal CVD (Chemical Vapor Deposition), photo- 20 CVD or plasma CVD. Among them, plasma CVD is suitably employed, in which gaseous raw materials are decomposed through application of direct current or high-frequency or microwave glow discharge to form an a-Si deposition film on the support.

25 The shape of the electrostatic latent image bearing member is not particularly limited and may be appropriately selected depending on the intended purpose, but it is preferably a hollow-cylindrical shape. The outer diameter of the electrostatic latent image bearing member having a hollow- 30 cylindrical shape is not particularly limited and may be appropriately selected depending on the intended purpose, but it is preferably 3 mm to 100 mm, more preferably 5 mm to 50 mm, particularly preferably 10 mm to 30 mm.

<Electrostatic Latent Image Forming Unit and Electrostatic Latent Image Forming Step>

The electrostatic latent image forming unit is not particularly limited and may be appropriately selected depending on the intended purpose so long as it is a unit configured to form an electrostatic latent image on the electrostatic latent 40 image bearing member. Examples thereof include a unit including at least a charging member configured to charge a surface of the electrostatic latent image bearing member and an exposing member configured to imagewise expose the surface of the electrostatic latent image bearing member to light.

45 The electrostatic latent image forming step is not particularly limited and may be appropriately selected depending on the intended purpose so long as it is a step of forming an electrostatic latent image on the electrostatic latent image bearing member. The electrostatic latent image forming step can be performed using the electrostatic latent image forming unit by, for example, charging a surface of the electrostatic latent image bearing member and then imagewise exposing the surface thereof to light.

55 -Charging Member and Charging-

The charging member is not particularly limited and may be appropriately selected depending on the intended purpose. Examples thereof include contact-type charging devices known per se having, for example, an electrically 60 conductive or semiconductive roller, brush, film and rubber blade; and non-contact-type charging devices utilizing corona discharge such as corotron and scorotron.

The charging can be performed by, for example, applying voltage to the surface of the electrostatic latent image bearing member using the charging member.

65 The charging member may have any shape like a charging roller as well as a magnetic brush or a fur brush. The shape

31

thereof may be suitably selected according to the specification or configuration of the image forming apparatus.

The charging member is not limited to the aforementioned contact-type charging members. However, the contact-type charging members are preferably used from the viewpoint of producing an image forming apparatus in which the amount of ozone generated from the charging members is reduced.

-Exposing Member and Exposure-

The exposing member is not particularly limited and may be appropriately selected depending on the purpose so long as it attains desired imagewise exposure on the surface of the electrophotographic latent image bearing member charged with the charging member. Examples thereof include various exposing members such as a copy optical exposing device, a rod lens array exposing device, a laser optical exposing device, and a liquid crystal shutter exposing device.

A light source used for the exposing member is not particularly limited and may be appropriately selected depending on the intended purpose. Examples thereof include conventional light-emitting devices such as a fluorescent lamp, a tungsten lamp, a halogen lamp, a mercury lamp, a sodium lamp, a light-emitting diode (LED), a laser diode (LD) and an electroluminescence (EL) device.

Also, various filters may be used for emitting only light having a desired wavelength range. Examples of the filters include a sharp-cut filter, a band-pass filter, an infrared cut filter, a dichroic filter, an interference filter and a color temperature conversion filter.

The exposure can be performed by, for example, imagewise exposing the surface of the electrostatic latent image bearing member to light using the exposing member.

In the present invention, light may be imagewise applied from the side facing the support of the electrostatic latent image bearing member.

<Developing Unit and Developing Step>

The developing unit is not particularly limited and may be appropriately selected depending on the intended purpose so long as it is a developing unit containing a toner for developing the electrostatic latent image formed on the electrostatic latent image bearing member to thereby form a visible image.

The developing step is not particularly limited and may be appropriately selected depending on the intended purpose so long as it is a step of developing the electrostatic latent image formed on the electrostatic latent image bearing member with a toner, to thereby form a visible image. The developing step can be performed by the developing unit.

The developing unit may employ a dry or wet developing process, and may be a single-color or multi-color developing unit.

The developing unit is preferably a developing device containing: a stirring device for charging the toner with friction generated during stirring; a magnetic field-generating unit fixed inside; and a developer bearing member configured to bear a developer containing the toner on a surface thereof and to be rotatable.

In the developing unit, toner particles and carrier particles are stirred and mixed so that the toner particles are charged by friction generated therebetween. The charged toner particles are retained in the chain-like form on the surface of the rotating magnetic roller to form magnetic brushes. The magnetic roller is disposed proximately to the electrostatic latent image developing member and thus, some of the toner particles forming the magnetic brushes on the magnet roller are transferred onto the surface of the electrostatic latent image developing member by the action of electrically

32

attractive force. As a result, the electrostatic latent image is developed with the toner particles to form a visual toner image on the surface of the electrostatic latent image developing member.

<Other Units and Other Steps>

Examples of the other units include a transfer unit, a fixing unit, a cleaning unit, a charge-eliminating unit, a recycling unit, and a controlling unit.

Examples of the other step include a transfer step, a fixing step, a cleaning step, a charge-eliminating step, a recycling step, and a controlling step.

-Transfer Unit and Transfer Step-

The transfer unit is not particularly limited and may be appropriately selected depending on the intended purpose so long as it is a unit configured to transfer the visible image onto a recording medium. Preferably, the transfer unit includes: a primary transfer unit configured to transfer the visible images to an intermediate transfer member to form a composite transfer image; and a secondary transfer unit configured to transfer the composite transfer image onto a recording medium.

The transfer step is not particularly limited and may be appropriately selected depending on the intended purpose so long as it is a step of transferring the visible image onto a recording medium. In this step, preferably, the visible images are primarily transferred to an intermediate transfer member, and the thus-transferred visible images are secondarily transferred to the recording medium.

For example, the transfer step can be performed using the transfer unit by charging the photoconductor with a transfer charger to transfer the visible image.

Here, when the image to be secondarily transferred onto the recording medium is a color image of several color toners, a configuration can be employed in which the transfer unit sequentially superposes the color toners on top of another on the intermediate transfer member to form an image on the intermediate transfer member, and the image on the intermediate transfer member is secondarily transferred at one time onto the recording medium by the intermediate transfer unit.

The intermediate transfer member is not particularly limited and may be appropriately selected from known transfer members depending on the intended purpose. For example, the intermediate transfer member is preferably a transferring belt.

The transfer unit (including the primary- and secondary transfer units) preferably includes at least a transfer device which transfers the visible images from the photoconductor onto the recording medium. Examples of the transfer device include a corona transfer device employing corona discharge, a transfer belt, a transfer roller, a pressing transfer roller and an adhesive transferring device.

The recording medium is not particularly limited and may be appropriately selected depending on the purpose, so long as it can receive a developed, unfixed image. Examples of the recording medium include plain paper and a PET base for OHP, with plain paper being used typically.

-Fixing Unit and Fixing Step-

The fixing unit is not particularly limited and may be appropriately selected depending on the intended purpose as long as it is a unit configured to fix a transferred image which has been transferred on the recording medium, but is preferably known heating-pressurizing members. Examples thereof include a combination of a heat roller and a press roller, and a combination of a heat roller, a press roller and an endless belt.

The fixing step is not particularly restricted and may be appropriately selected according to purpose, as long as it is a step of fixing a visible image which has been transferred on the recording medium. The fixing step may be performed every time when an image of each color toner is transferred onto the recording medium, or at one time (at the same time) on a laminated image of color toners.

The fixing step can be performed by the fixing unit.

The heating-pressurizing member usually performs heating preferably at 80° C. to 200° C.

Notably, in the present invention, known photofixing devices may be used instead of or in addition to the fixing unit depending on the intended purpose.

A surface pressure at the fixing step is not particularly limited and may be appropriately selected depending on the intended purpose, but is preferably 10 N/cm<sup>2</sup> to 80 N/cm<sup>2</sup>.

#### -Cleaning Unit and Cleaning Step-

The cleaning unit is not particularly limited and may be appropriately selected depending on the intended purpose, as long as it can remove the toner remaining on the photoconductor. Examples thereof include a magnetic brush cleaner, an electrostatic brush cleaner, a magnetic roller cleaner, a blade cleaner, a brush cleaner and a web cleaner.

The cleaning step is not particularly limited and may be appropriately selected depending on the intended purpose, as long as it is a step of removing the toner remaining on the photoconductor. It may be performed by the cleaning unit.

#### -Charge-Eliminating Unit and Charge-Eliminating Step-

The charge-eliminating unit is not particularly limited and may be appropriately selected depending on the intended purpose, as long as it is a unit configured to apply a charge-eliminating bias to the photoconductor to thereby charge-eliminate. Example thereof includes a charge-eliminating lamp.

The charge-eliminating step is not particularly limited and may be appropriately selected depending on the intended purpose, as long as it is a step of applying a charge-eliminating bias to the photoconductor to thereby charge-eliminate. It may be carried out by the charge-eliminating unit.

#### -Recycling Unit and Recycling Step-

The recycling unit is not particularly limited and may be appropriately selected depending on the intended purpose, as long as it is a unit configured to recycle the toner which has been removed at the cleaning step to the developing device. Examples thereof include a known conveying unit.

The recycling step is not particularly limited and may be appropriately selected depending on the intended purpose, as long as it is a step of recycling the toner which has been removed at the cleaning step to the developing device. The recycling step can be performed by the recycling unit.

#### -Control Unit and Control Step-

The control unit is not particularly limited and may be appropriately selected depending on the intended purpose, as long as it can control the operation of each of the above units. Examples thereof include devices such as sequencer and computer.

The control step is not particularly limited and may be appropriately selected depending on the intended purpose, as long as it is a step of controlling the operation of each of the above units. The control step can be performed by the control unit.

One embodiment for performing an image forming method by an image forming apparatus of the present invention now will be explained with reference to FIG. 1. An image forming apparatus 100A illustrated in FIG. 1 includes a photoconductor drum 10 serving as the electrostatic latent

image bearing member (hereinafter may be referred to as a "photoconductor 10"), a charging roller 20 serving as the charging unit, an exposing device 30 serving as the exposing unit, a developing device 40 serving as the developing unit, an intermediate transfer member 50, a cleaning device 60 serving as the cleaning unit which includes a cleaning blade and a charge-eliminating lamp 70 serving as the charge-eliminating unit.

The intermediate transfer member 50 is an endless belt 10 and designed so as to be movable in a direction indicated by an arrow by three rollers 51 which are disposed inside the belt and around which the belt is stretched. A part of the three rollers 51 also functions as a transfer bias roller which may apply a predetermined transfer bias (primary transfer bias) to the intermediate transfer member 50. Also, a cleaning device 90 including a cleaning blade is disposed near the intermediate transfer member 50. Further, a transfer roller 80 serving as the transfer unit which can apply a transfer bias for transferring (secondary transferring) a developed image 20 (toner image) onto transfer paper 95 serving as a recording medium is disposed near the intermediate transfer member 50 facing the intermediate transfer member 50. In addition, around the intermediate transfer member 50, a corona charging device 58 for applying a charge to the toner image transferred on the intermediate transfer member 50 is disposed between a contact portion of the electrostatic latent image bearing member 10 with the intermediate transfer member 50 and a contact portion of the intermediate transfer member 50 with the transfer paper 95 in a rotational direction 25 of the intermediate transfer member 50.

The developing device 40 includes a developing belt 41 serving as the developer bearing member; and a black developing unit 45K, a yellow developing unit 45Y, a magenta developing unit 45M and a cyan developing unit 45C which are arranged around the developing belt 41. Here, the black developing unit 45K includes a developer container 42K, a developer supply roller 43K and a developing roller 44K. The yellow developing unit 45Y includes a developer container 42Y, a developer supply roller 43Y and a developing roller 44Y. The magenta developing unit 45M includes a developer container 42M, a developer supply roller 43M and a developing roller 44M. The cyan developing unit 45C includes a developer container 42C, a developer supply roller 43C and a developing roller 44C. 45 Also, the developing belt 41 is an endless belt which is rotatably stretched around a plurality of belt rollers and is partially in contact with the electrostatic latent image bearing member 10.

In the color image forming apparatus 100A illustrated in FIG. 1, the charging roller 20 uniformly charges a surface of the photoconductor drum 10, and then the exposing device 30 imagewise-exposes the photoconductor drum 10 to form an electrostatic latent image. Next, the electrostatic latent image formed on the photoconductor drum 10 is developed 50 with a toner supplied from the developing device 40 to form a toner image. Further, the toner image is transferred (primarily transferred) onto the intermediate transfer member 50 by voltage applied from the roller 51 and then transferred (secondarily transferred) onto transfer paper 95. As a result, a transferred image is formed on the transfer paper 95. Notably, a residual toner remaining on the photoconductor drum 10 is removed by the cleaning device 60, and the photoconductor drum 10 is once charge-eliminated by the charge-eliminating lamp 70.

FIG. 2 is a schematic structural view of another example of an image forming apparatus of the present invention. An image forming apparatus 100B has the same configuration

as the image forming apparatus 100A illustrated in FIG. 1 except that the developing belt 41 is not included and that, around the photoconductor drum 10, the black developing unit 45K, the yellow developing unit 45Y, the magenta developing unit 45M and the cyan developing unit 45C are disposed facing directly to the electrostatic latent image bearing member.

FIG. 3 is a schematic structural view of still another example of an image forming apparatus of the present invention. The color image forming apparatus illustrated in FIG. 3 includes a copying device main body 150, a paper feeding table 200, a scanner 300 and an automatic document feeder (ADF) 400.

An intermediate transfer member 50 which is an endless belt is disposed at a central part of the copying device main body 150. The intermediate transfer member 50 is stretched around support rollers 14, 15 and 16 and can rotate in a clockwise direction in FIG. 3. Near the support roller 15, a cleaning device for the intermediate transfer member 17 is disposed to remove a residual toner remaining on the intermediate transfer member 50. On the intermediate transfer member 50 stretched around the support rollers 14 and 15, a tandem type developing device 120 is disposed in which four image forming units 18 of yellow, cyan, magenta and black are arranged in parallel so as to face to each other along a conveying direction thereof. The exposing device 21 serving as the exposing member is disposed in proximity to the tandem type developing device 120. Further, a secondary transfer device 22 is disposed on a side of the intermediate transfer member 50 opposite to the side on which the tandem type developing device 120 is disposed. In the secondary transfer device 22, the secondary transfer belt 24 which is an endless belt is stretched around a pair of rollers 23, and the transfer paper conveyed on the secondary transfer belt 24 and the intermediate transfer member 50 may contact with each other. Here, a fixing device 25 serving as the fixing unit is disposed in proximity to the secondary transfer device 22. The fixing device 25 includes a fixing belt 26 which is an endless belt and a press roller 27 which is disposed so as to be pressed against the fixing belt.

Here, in the tandem type image forming apparatus, a sheet inverting device 28 is disposed near the secondary transfer device 22 and the fixing device 25 for inverting the transfer paper in the case of forming images on both sides of the transfer paper.

Next, a method for forming a full-color image (color-copying) using the tandem type developing device 120 will be explained. First, a color document is set on a document table 130 of the automatic document feeder (ADF) 400. Alternatively, the automatic document feeder 400 is opened, the color document is set on a contact glass 32 of the scanner 300, and the automatic document feeder 400 is closed.

When a start button (not shown) is pressed, the scanner 300 activates after the color document is conveyed and moved to the contact glass 32 in the case the color document has been set on the automatic document feeder 400, or right away in the case the color document has been set on the contact glass 32, so that a first travelling body 33 and a second travelling body 34 travel. At this time, a light is irradiated from a light source in the first travelling body 33, the light reflected from a surface of the document is reflected by a mirror in the second travelling body 34 and then is received by a reading sensor 36 through an imaging lens 35. Thus, the color document (color image) is read to thereby form black, yellow, magenta and cyan image information.

The image information of black, yellow, magenta, and cyan are transmitted to the image forming units 18 (black

image forming unit, yellow image forming unit, magenta image forming unit, and cyan image forming unit) in the tandem type developing device 120, and toner images of black, yellow, magenta, and cyan are formed in the image forming units. As illustrated in FIG. 4, the image forming units 18 (black image forming unit, yellow image forming unit, magenta image forming unit, and cyan image forming unit) in the tandem type developing device 120 include: electrostatic latent image bearing members 10 (black electrostatic latent image bearing member 10K, yellow electrostatic latent image bearing member 10Y, magenta electrostatic latent image bearing member 10M, and cyan electrostatic latent image bearing member 10C); a charging device 160 configured to uniformly charge the electrostatic latent image bearing members 10; an exposing device configured to imagewise-expose to a light (L illustrated in FIG. 4) the electrostatic latent image bearing members based on color image information to form an electrostatic latent image corresponding to color images on the electrostatic latent image bearing members; a developing device 61 configured to develop the electrostatic latent images with color toners (black color toner, yellow color toner, magenta color toner, and cyan color toner) to form a toner image of the color toners; a transfer charger 62 configured to transfer the toner image onto the intermediate transfer member 50; a cleaning device 63; and a charge-eliminating unit 64. Each image forming unit 18 can form monochrome images (black image, yellow image, magenta image, and cyan image) based on image formations of colors. Thus formed black image (i.e., black image formed onto the black electrostatic latent image bearing member 10K), yellow image (i.e., yellow image formed onto the yellow electrostatic latent image bearing member 10Y), magenta image (i.e., magenta image formed onto the magenta electrostatic latent image bearing member 10M), and cyan image (i.e., cyan image formed onto the cyan electrostatic latent image bearing member 10C) are sequentially transferred (primarily transferred) onto the intermediate transfer member 50 which is rotatably moved by the support rollers 14, 15 and 16. The black image, the yellow image, the magenta image, and the cyan image are superposed on the intermediate transfer member 50 to thereby form a composite color image (color transfer image).

Meanwhile, on the paper feeding table 200, one of paper feeding rollers 142 is selectively rotated to feed a sheet (recording paper) from one of the paper feeding cassettes 144 equipped in multiple stages in a paper bank 143. The sheet is separated one by one by a separation roller 145 and sent to a paper feeding path 146. The sheet (recording paper) is conveyed by a conveying roller 147 and is guided to a paper feeding path 148 in the copying device main body 150, and stops by colliding with a registration roller 49. Alternatively, a paper feeding roller 142 is rotated to feed a sheet (recording paper) on a manual feed tray 54. The sheet (recording paper) is separated one by one by a separation roller 52 and is guided to a manual paper feeding path 53, and stops by colliding with the registration roller 49. Notably, the registration roller 49 is generally used while grounded, but it may also be used in a state that a bias is being applied for removing paper dust on the sheet. Next, by rotating the registration roller 49 in accordance with the timing of the composite toner image (color transferred image) formed on the intermediate transfer member 50, the sheet (recording paper) is fed to between the intermediate transfer member 50 and the secondary transfer device 22. Thereby, the composite toner image (color transferred image) is transferred (secondarily transferred) by the sec-

ondary transfer device 22 onto the sheet (recording paper) to thereby form a color image on the sheet (recording paper). Notably, a residual toner remaining on the intermediate transfer member 50 after image transfer is removed by the cleaning device for the intermediate transfer member 17.

The sheet (recording paper) on which the color image has been transferred is conveyed by the secondary transfer device 22, and then conveyed to the fixing device 25. In the fixing device 25, the composite color image (color transferred image) is fixed on the sheet (recording paper) by the action of heat and pressure. Next, the sheet (recording paper) is switched by a switching claw 55, and discharged by a discharge roller 56 and stacked in a paper discharge tray 57. Alternatively, the sheet is switched by the switching claw 55, and is inverted by the inverting device 28 to thereby be guided to a transfer position again. After an image is formed similarly on the rear surface, the recording paper is discharged by the discharge roller 56 stacked in the paper discharge tray 57.

(Process Cartridge)

A process cartridge of the present invention is molded so as to be mounted to various image forming apparatuses in an attachable and detachable manner, including at least an electrostatic latent image bearing member configured to bear an electrostatic latent image thereon; and a developing unit configured to develop the electrostatic latent image borne on the electrostatic latent image bearing member with the developer of the present invention to form a toner image. Note that, the process cartridge of the present invention may further include other units, if necessary.

The developing unit includes at least a developer accommodating container that accommodates the developer of the present invention, and a developer bearing member configured to bear and transfer the developer accommodated in the developer accommodating container. Note that, the developing unit may further include, for example, a regulating member configured to regulate the thickness of the borne developer.

FIG. 5 illustrates one example of the process cartridge of the present invention. A process cartridge 110 includes a photoconductor drum 10, a corona charging device 58, a developing device 40, a transfer roller 80, and a cleaning device 90.

## EXAMPLES

The present invention will be described by way of Examples below. The present invention should not be construed as being limited to the Examples. Unless otherwise specified, "part(s)" means "part(s) by mass". Unless otherwise specified, "%" means "% by mass".

Measurements in the Examples below were obtained by the methods described in the present specification. Note that, the Tg and molecular weights of the non-crystalline polyester resin A, the non-crystalline polyester resin B, and the crystalline polyester resin C and the like were measured from each resin obtained in Production Example.

### Production Example 1

#### Synthesis of Ketimine

A reaction vessel to which a stirring bar and a thermometer had been set was charged with 170 parts of isophorone diamine and 75 parts of methyl ethyl ketone, and the resulting mixture was allowed to react for 5 hours at 50° C.,

to thereby obtain [ketimine compound 1]. The [ketimine compound 1] was found to have an amine value of 418.

### Production Example A-1

#### Synthesis of Non-Crystalline Polyester Resin A-1

##### Synthesis of Prepolymer A-1-

A reaction vessel equipped with a condenser, a stirrer and a nitrogen-introducing tube was charged with 3-methyl-1, 5-pentanediol, isophthalic acid, and adipic acid so that the molar ratio of hydroxyl groups to carboxyl groups, represented by OH/COOH, was 1.1, the diol component was composed of 100 mol % of 3-methyl-1,5-pentanediol, the dicarboxylic acid component was composed of 45 mol % of isophthalic acid, and 55 mol % of adipic acid, and an amount of trimethylol propane was 1.5 mol % relative to the total amount of the monomers, together with titanium tetrakisopropoxide (1,000 ppm relative to the resin component).

10 Thereafter, the mixture was heated to 200° C. over about 4 hours, and heated to 230° C. over 2 hours, followed by carrying out a reaction until effluent water stopped. Thereafter, the resultant was allowed to further react for 5 hours under the reduced pressure of 10 mmHg to 15 mmHg, to thereby yield intermediate polyester A-1.

15 Next, a reaction vessel equipped with a condenser, a stirrer and a nitrogen-introducing tube was charged with the obtained intermediate polyester A-1, and isophorone diisocyanate (IPDI) at a molar ratio (isocyanate groups of IPDI/ hydroxyl groups of intermediate polyester) of 2.0, and after diluted with ethyl acetate to give a 50% ethyl acetate solution, the mixture was allowed to react for 5 hours at 100° C., to thereby obtain [prepolymer A-1].

##### Synthesis of Non-Crystalline Polyester Resin A-1-

20 The obtained prepolymer A-1 was stirred in a reaction vessel equipped with a heating device, a stirrer, and a nitrogen-introducing tube, and into the reaction vessel, the [ketimine compound 1] was added dropwise so that the amount of the amine of the [ketimine compound 1] was equimolar to the amount of the isocyanate of the prepolymer A-1. After stirring for 10 hours at 45° C., a resulting prepolymer elongated product was taken out. The obtained prepolymer elongated product was dried at 50° C. under reduced pressure until the amount of the ethyl acetate residues in the prepolymer elongated product became 100 ppm or less, to thereby obtain non-crystalline polyester resin A-1. This resin was found to have a weight average molecular weight (Mw) of 164,000 and a Tg of -40° C.

### Production Example A-2

#### Synthesis of Non-Crystalline Polyester Resin A-2

##### Synthesis of Prepolymer A-2-

25 A reaction vessel equipped with a condenser, a stirrer and a nitrogen-introducing tube was charged with 3-methyl-1, 5-pentanediol and adipic acid so that the molar ratio of hydroxyl groups to carboxyl groups, represented by OH/COOH, was 1.1, the diol component was composed of 100 mol % of 3-methyl-1,5-pentanediol, the dicarboxylic acid component was composed of 80 mol % of adipic acid and 20 mol % of adipic acid, and an amount of trimethylolpropane was 1.5 mol % relative to a total amount of the monomers, together with titanium tetrakisopropoxide (1,000 ppm relative to the resin component). Thereafter, the mixture was heated to 200° C. over about 4 hours, and heated to 230° C. over 2 hours, followed by carrying out a reaction

until effluent water stopped. Thereafter, the resultant was allowed to further react for 5 hours under the reduced pressure of 10 mmHg to 15 mmHg, to thereby yield intermediate polyester A-2.

Next, a reaction vessel equipped with a condenser, a stirrer and a nitrogen-introducing tube was charged with the obtained intermediate polyester A-2, and isophorone diisocyanate (IPDI) at a molar ratio (isocyanate groups of IPDI/hydroxyl groups of intermediate polyester) of 2.0, and after diluted with ethyl acetate to give a 50% ethyl acetate solution, the mixture was allowed to react for 5 hours at 100° C., to thereby obtain prepolymer A-2.

**-Synthesis of Non-Crystalline Polyester Resin A-2-**

The obtained prepolymer A-2 was stirred in a reaction vessel equipped with a heating device, stirrer, and nitrogen inlet tube, and into the reaction vessel, the [ketimine compound 1] was added dropwise so that the amount of the amine of [ketimine compound 1] was equimolar to the amount of the isocyanate of the prepolymer A-2. After stirring for 10 hours at 45° C., a resulting prepolymer elongated product was taken out. The obtained prepolymer elongated product was dried at 50° C. under reduced pressure until the amount of the ethyl acetate residues in the prepolymer elongated product became 100 ppm or less, to thereby obtain non-crystalline polyester resin A-2. This resin was found to have a weight average molecular weight (Mw) of 175,000 and a Tg of -55° C.

**Production Example A-3**

**Synthesis of Non-Crystalline Polyester Resin A-3**

**-Synthesis of Prepolymer A-3-**

A reaction vessel equipped with a condenser, a stirrer and a nitrogen-introducing tube was charged with bisphenol A ethylene oxide 2 mol adduct, bisphenol A propylene oxide 2 mol adduct, terephthalic acid, and trimellitic anhydride so that the molar ratio of hydroxyl groups to carboxyl groups, represented by OH/COOH, was 1.3, the diol component was composed of 90 mol % of bisphenol A ethylene oxide 2 mol adduct and 10 mol % of bisphenol A propylene oxide 2 mol adduct, and the dicarboxylic acid was composed of 90 mol % of terephthalic acid and 10 mol % of trimellitic anhydride, together with titanium tetraisopropoxide (1,000 ppm relative to the resin component). Thereafter, the mixture was heated to 200° C. over about 4 hours, and heated to 230° C. over 2 hours, followed by carrying out a reaction until effluent water stopped. Thereafter, the resultant was allowed to further react for 5 hours under the reduced pressure of 10 mmHg to 15 mmHg, to thereby yield intermediate polyester A-3.

Next, a reaction vessel equipped with a condenser, a stirrer and a nitrogen-introducing tube was charged with intermediate polyester A-3, and isophorone diisocyanate (IPDI) at a molar ratio (isocyanate groups of IPDI/hydroxyl groups of intermediate polyester) of 2.0, and after diluted with ethyl acetate to give a 50% ethyl acetate solution, the mixture was allowed to react for 5 hours at 100° C., to thereby obtain prepolymer A-3.

**-Synthesis of Non-Crystalline Polyester Resin A-3-**

The obtained prepolymer A-3 was stirred in a reaction vessel equipped with a heating device, stirrer, and nitrogen inlet tube, and into the reaction vessel, the [ketimine compound 1] was added dropwise so that the amount of the amine of the [ketimine compound 1] was equimolar to the amount of the isocyanate of the prepolymer A-3. After stirring for 10 hours at 45° C., a resulting prepolymer

elongated product was taken out. The obtained prepolymer elongated product was dried at 50° C. under reduced pressure until the amount of the ethyl acetate residues in the prepolymer elongated product became 100 ppm or less, to thereby obtain non-crystalline polyester resin A-3. This resin was found to have a weight average molecular weight (Mw) of 130,000 and a Tg of 54° C.

**Production Example A-4**

**Synthesis of Non-Crystalline Polyester Resin A-4**

**-Synthesis of Prepolymer A-4-**

A reaction vessel equipped with a condenser, a stirrer and a nitrogen-introducing tube was charged with 1,2-propylene glycol, terephthalic acid, adipic acid, and trimellitic anhydride so that the molar ratio of hydroxyl groups to carboxyl groups, represented by OH/COOH, was 1.3, the diol component was composed of 100 mol % of 1,2-propylene glycol, the dicarboxylic acid component was composed of 80 mol % of terephthalic acid and 20 mol % of adipic acid, and an amount of trimellitic anhydride was 2.5 mol % relative to the total amount of the monomers, together with titanium tetraisopropoxide (1,000 ppm relative to the resin component). Thereafter, the mixture was heated to 200° C. over about 4 hours, and heated to 230° C. over 2 hours, followed by carrying out a reaction until effluent water stopped. Thereafter, the resultant was allowed to further react for 5 hours under the reduced pressure of 10 mmHg to 15 mmHg, to thereby yield intermediate polyester A-4.

Next, a reaction vessel equipped with a condenser, a stirrer and a nitrogen-introducing pipe was charged with the obtained intermediate polyester A-4, and isophorone diisocyanate (IPDI) at a molar ratio (isocyanate groups of IPDI/hydroxyl groups of intermediate polyester) of 2.0, and after diluted with ethyl acetate to give a 50% ethyl acetate solution, the mixture was allowed to react for 5 hours at 100° C., to thereby obtain prepolymer A-4.

**-Synthesis of Non-Crystalline Polyester Resin A-4-**

The obtained prepolymer A-4 was stirred in a reaction vessel equipped with a heating device, stirrer, and nitrogen inlet tube, and into the reaction vessel, the [ketimine compound 1] was added dropwise so that the amount of the amine of the [ketimine compound 1] was equimolar to the amount of the isocyanate of the prepolymer A-4. After stirring for 10 hours at 45° C., a resulting prepolymer elongated product was taken out. The obtained prepolymer elongated product was dried at 50° C. under reduced pressure until the amount of the ethyl acetate residues in the prepolymer elongated product became 100 ppm or less, to thereby obtain non-crystalline polyester resin A-4. This resin was found to have a weight average molecular weight (Mw) of 140,000 and a Tg of 56° C.

**Production Example A-5**

**Synthesis of Non-Crystalline Polyester Resin A-5**

**-Synthesis of Prepolymer A-5-**

A reaction vessel equipped with a condenser, a stirrer and a nitrogen-introducing tube was charged with 3-methyl-1,5-pentanediol, isophthalic acid, adipic acid, and trimellitic anhydride so that the molar ratio of hydroxyl groups to carboxyl groups, represented by OH/COOH, was 1.5, the diol component was composed of 100 mol % of 3-methyl-1,5-pentanediol, the dicarboxylic acid component was composed of 40 mol % of isophthalic acid and 60 mol % of

41

adipic acid, and an amount of trimellitic anhydride was 1 mol % relative to the total amount of the monomers, together with titanium tetraisopropoxide (1,000 ppm relative to the resin component). Thereafter, the mixture was heated to 200° C. over about 4 hours, and heated to 230° C. over 2 hours, followed by carrying out a reaction until effluent water stopped. Thereafter, the resultant was allowed to further react for 5 hours under the reduced pressure of 10 mmHg to 15 mmHg, to thereby yield intermediate polyester A-5.

Next, a reaction vessel equipped with a condenser, a stirrer and a nitrogen-introducing pipe was charged with the obtained intermediate polyester A-5, and isophorone diisocyanate (IPDI) at a molar ratio (isocyanate groups of IPDI/ hydroxyl groups of intermediate polyester) of 2.0, and after diluted with ethyl acetate to give a 50% ethyl acetate solution, the mixture was allowed to react for 5 hours at 100° C., to thereby obtain prepolymer A-5.

-Synthesis of Non-Crystalline Polyester Resin A-5-

The obtained prepolymer A-5 was stirred in a reaction vessel equipped with a heating device, stirrer, and nitrogen inlet tube, and into the reaction vessel, the [ketimine compound 1] was added dropwise so that the amount of the amine of the [ketimine compound 1] was equimolar to the amount of the isocyanate of the prepolymer A-5. After stirring for 10 hours at 45° C., a resulting prepolymer elongated product was taken out. The obtained prepolymer elongated product was dried at 50° C. under reduced pressure until the amount of the ethyl acetate residues in the prepolymer elongated product became 100 ppm or less, to thereby obtain non-crystalline polyester resin A-5. This resin was found to have a weight average molecular weight (Mw) of 150,000 and a Tg of -35° C.

Production Example A-6

Synthesis of Non-Crystalline Polyester Resin A-6

-Synthesis of Prepolymer A-6-

A reaction vessel equipped with a condenser, a stirrer and a nitrogen-introducing pipe was charged with 1,6-hexanediol, isophthalic acid, adipic acid, and trimellitic anhydride so that the molar ratio of hydroxyl groups to carboxyl groups, represented by OH/COOH, was 1.5, the diol component was composed of 100 mol % of 1,6-hexanediol, the dicarboxylic acid component was composed of 80 mol % of isophthalic acid and 20 mol % of adipic acid, and an amount of trimellitic anhydride was 1 mol % relative to the total amount of the monomers, together with titanium tetraisopropoxide (1,000 ppm relative to the resin component). Thereafter, the mixture was heated to 200° C. over about 4 hours, and heated to 230° C. over 2 hours, followed by carrying out a reaction until effluent water stopped. Thereafter, the resultant was allowed to further react for 5 hours under the reduced pressure of 10 mmHg to 15 mmHg, to thereby yield intermediate polyester A-6.

Next, a reaction vessel equipped with a condenser, a stirrer and a nitrogen-introducing pipe was charged with the obtained intermediate polyester A-6, and isophorone diisocyanate (IPDI) at a molar ratio (isocyanate groups of IPDI/ hydroxyl groups of intermediate polyester) of 2.0, and after diluted with ethyl acetate to give a 50% ethyl acetate solution, the mixture was allowed to react for 5 hours at 100° C., to thereby obtain prepolymer A-6.

-Synthesis of Non-Crystalline Polyester Resin A-6-

The obtained prepolymer A-6 was stirred in a reaction vessel equipped with a heating device, stirrer, and nitrogen

42

inlet tube, and into the reaction vessel, the [ketimine compound 1] was added dropwise so that the amount of the amine of [ketimine compound 1] was equimolar to the amount of the isocyanate of the prepolymer A-6. After stirring for 10 hours at 45° C., a resulting prepolymer elongated product was taken out. The obtained prepolymer elongated product was dried at 50° C. under reduced pressure until the amount of the ethyl acetate residues in the prepolymer elongated product became 100 ppm or less, to thereby obtain non-crystalline polyester resin A-6. This resin was found to have a weight average molecular weight (Mw) of 120,000 and a Tg of -5° C.

Production Example B-1

Synthesis of Non-Crystalline Polyester Resin B-1

A four necked flask equipped with a nitrogen-introducing tube, a drainpipe, a stirrer and a thermocouple was charged with bisphenol A ethylene oxide 2 mol adduct, bisphenol A propylene oxide 2 mol adduct, terephthalic acid, and adipic acid, so that the molar ratio of the bisphenol A propylene oxide 2 mol adduct to the bisphenol A ethylene oxide 2 mol adduct (bisphenol A propylene oxide 2 mol adduct/bisphenol A ethylene oxide 2 mol adduct) was 60/40, the molar ratio of terephthalic acid to adipic acid (terephthalic acid/adipic acid) was 97/3, and the molar ratio of hydroxyl groups to carboxyl groups, represented by OH/COOH, was 1.3. The resulting mixture was allowed to react with titanium tetraisopropoxide (500 ppm relative to the resin component) for 8 hours at 230° C. under atmospheric pressure, and was further reacted for 4 hours under the reduced pressure of 10 mmHg to 15 mmHg. Thereafter, trimellitic anhydride was added to the reaction vessel in an amount of 1 mol % relative to the entire resin component, and the resultant was allowed to react for 3 hours at 180° C., under atmospheric pressure, to thereby obtain non-crystalline polyester resin B-1. This resin was found to have a weight average molecular weight (Mw) of 5,300 and a Tg of -67° C.

Production Example B-2

Synthesis of Non-Crystalline Polyester Resin B-2

A four necked flask equipped with a nitrogen-introducing tube, a drainpipe, a stirrer and a thermocouple was charged with bisphenol A ethylene oxide 2 mol adduct, 1,3-propylene glycol, terephthalic acid, and adipic acid so that the molar ratio of the bisphenol A propylene oxide 2 mol adduct to the 1,3-propylene glycol (bisphenol A propylene oxide 2 mol adduct/1,3-propylene glycol) was 90/10, the molar ratio of terephthalic acid to adipic acid (terephthalic acid/adipic acid) was 80/20, and the molar ratio of hydroxyl groups to carboxyl groups, represented by OH/COOH, was 1.4. The resulting mixture was allowed to react with titanium tetraisopropoxide (500 ppm relative to the resin component) for 8 hours at 230° C. under atmospheric pressure, and was further reacted for 4 hours under the reduced pressure of 10 mmHg to 15 mmHg. Thereafter, trimellitic anhydride was added to the reaction vessel in an amount of 1 mol % relative to the entire resin component, and the resultant was allowed to react for 3 hours at 180° C., under atmospheric pressure, to thereby obtain non-crystalline polyester resin B-2. This resin was found to have a weight average molecular weight (Mw) of 5,600 and a Tg of 61° C.

## Production Example B-3

## Synthesis of Non-Crystalline Polyester Resin B-3

A four necked flask equipped with a nitrogen-introducing tube, a drainpipe, a stirrer and a thermocouple was charged with bisphenol A propylene oxide 2 mol adduct, bisphenol A ethylene oxide 2 mol adduct, isophthalic acid, and adipic acid, so that the molar ratio of the bisphenol A propylene oxide 2 mol adduct to the bisphenol A ethylene oxide 2 mol adduct (bisphenol A propylene oxide 2 mol adduct/bisphenol A ethylene oxide 2 mol adduct) was 30/70, the molar ratio of isophthalic acid to adipic acid (isophthalic acid/adipic acid) was 80/20, and the molar ratio of hydroxyl groups to carboxyl groups, represented by OH/COOH, was 1.2. The resulting mixture was allowed to react with titanium tetrakisopropoxide (500 ppm relative to the resin component) for 8 hours at 230° C. under atmospheric pressure, and was further reacted for 4 hours under the reduced pressure of 10 mmHg to 15 mmHg. Thereafter, trimellitic anhydride was added to the reaction vessel in an amount of 1 mol % relative to the entire resin component, and the resultant was allowed to react for 3 hours at 180° C., under atmospheric pressure, to thereby obtain non-crystalline polyester resin B-3. This resin was found to have a weight average molecular weight (Mw) of 5,500 and a Tg of 50° C.

## Production Example B-4

## Synthesis of Non-Crystalline Polyester Resin B-4

A four necked flask equipped with a nitrogen-introducing pipe, a drainpipe, a stirrer and a thermocouple was charged with bisphenol A ethylene oxide 2 mol adduct, bisphenol A propylene oxide 3 mol adduct, isophthalic acid, and adipic acid, so that the molar ratio of the bisphenol A ethylene oxide 2 mol adduct to the bisphenol A propylene oxide 3 mol adduct (bisphenol A ethylene oxide 2 mol adduct/bisphenol A propylene oxide 3 mol adduct) was 85/15, the molar ratio of isophthalic acid to adipic acid (isophthalic acid/adipic acid) was 80/20, and the molar ratio of hydroxyl groups to carboxyl groups, represented by OH/COOH, was 1.3. The resulting mixture was allowed to react with titanium tetrakisopropoxide (500 ppm relative to the resin component) for 8 hours at 230° C. under atmospheric pressure, and was further reacted for 4 hours under the reduced pressure of 10 mmHg to 15 mmHg. Thereafter, trimellitic anhydride was added to the reaction vessel in an amount of 1 mol % relative to the entire resin component, and the resultant was allowed to react for 3 hours at 180° C., under atmospheric pressure, to thereby obtain non-crystalline polyester resin B-4. This resin was found to have a weight average molecular weight (Mw) of 5,000 and a Tg of 48° C.

## Production Example B-5

## Synthesis of Non-Crystalline Polyester Resin B-5

A four necked flask equipped with a nitrogen-introducing pipe, a drainpipe, a stirrer and a thermocouple was charged with bisphenol A ethylene oxide 2 mol adduct, bisphenol A propylene oxide 3 mol adduct, terephthalic acid, and adipic acid, so that the molar ratio of the bisphenol A ethylene oxide 2 mol adduct to the bisphenol A propylene oxide 3 mol adduct (bisphenol A ethylene oxide 2 mol adduct/bisphenol A propylene oxide 3 mol adduct) was 85/15, the molar ratio of terephthalic acid to adipic acid (terephthalic acid/adipic

acid) was 80/20, and the molar ratio of hydroxyl groups to carboxyl groups, represented by OH/COOH, was 1.3. The resulting mixture was allowed to react with titanium tetrakisopropoxide (500 ppm relative to the resin component) for 8 hours at 230° C. under atmospheric pressure, and was further reacted for 4 hours under the reduced pressure of 10 mmHg to 15 mmHg. Thereafter, trimellitic anhydride was added to the reaction vessel in an amount of 1 mol % relative to the entire resin component, and the resultant was allowed to react for 3 hours at 180° C., under atmospheric pressure, to thereby obtain non-crystalline polyester resin B-5. This resin was found to have a weight average molecular weight (Mw) of 5,000 and a Tg of 51° C.

15

## Production Example C-1

## Synthesis of Crystalline Polyester Resin C-1

A 5 L four necked flask equipped with a nitrogen-introducing pipe, a drainpipe, a stirrer and a thermocouple was charged with sebacic acid and 1,6-hexanediol, so that the molar ratio of hydroxyl groups to carboxyl groups, represented by OH/COOH, was 0.9. The resulting mixture was allowed to react with titanium tetrakisopropoxide (500 ppm relative to the resin component) for 10 hours at 180° C., and the heated to 200° C. and reacted for 3 hours, followed by further reacting for 2 hours under the pressure of 8.3 kPa, to thereby obtain crystalline polyester resin C-1. This resin was found to have a weight average molecular weight (Mw) of 25,000 and a Tg of 67° C.

35

## Example 1

## Preparation of Master Batch (MB)

Water (1,200 parts), 500 parts of carbon black (Printex 35, manufactured by Evonik Degussa Japan Co., Ltd.) [DBP oil absorption amount=42 mL/100 mg, pH=9.5], and 500 parts of the non-crystalline polyester resin B-1 were added and mixed together by means of HENSCHEL MIXER (manufactured by NIPPON COLE & ENGINEERING CO., LTD.), and the resulting mixture was kneaded by means of a two roll mill for 30 minutes at 150° C. The resulting kneaded product was rolled out and cooled, followed by pulverizing by a pulverizer, to thereby obtain master batch 1.

## &lt;Preparation of WAX Dispersion Liquid&gt;

A vessel to which a stirring bar and a thermometer had been set was charged with 50 parts of paraffin wax (HNP-9, manufactured by Nippon Seiro Co., Ltd., hydrocarbon wax, melting point: 75° C., SP value: 8.8) as releasing agent 1, and 450 parts of ethyl acetate, followed by heating to 80° C. with mixing. The temperature was maintained at 80° C. for 5 hours, followed by cooling to 30° C. over 1 hour. The

resulting mixture was dispersed by means of a bead mill (ULTRA VISCOMILL, product of AIMEX CO., Ltd.) under the conditions: a liquid feed rate of 1 kg/hr, disc circumferential velocity of 6 m/s, 0.5 mm-zirconia beads packed to 80% by volume, and 3 passes, to thereby obtain [WAX dispersion liquid 1].

## &lt;Preparation of Crystalline Polyester Resin Dispersion Liquid&gt;

A container equipped with a stirring bar and a thermometer was charged with 50 parts of the crystalline polyester resin C-1, and 450 parts of ethyl acetate, and the resulting mixture was heated to 80° C. with stirring. The temperature was kept at 80° C. for 5 hours, followed by cooling to 30°

45

C. over 1 hour. The resultant was dispersed by means of a bead mill (ULTRA VISCOMILL, manufactured by AIMEX CO., LTD.), under the following conditions: a liquid feed rate of 1 kg/hr, disc circumferential velocity of 6 m/s, zirconia beads 0.5 mm in diameter packed to 80% by volume, and 3 passes, to thereby obtain [crystalline polyester resin dispersion liquid 1].

<Preparation of Oil Phase>

A vessel was charged with 50 parts of the [WAX dispersion liquid 1], 150 parts of the [non-crystalline polyester resin A-1], 50 parts of the [crystalline polyester resin dispersion liquid 1], 750 parts of the [non-crystalline polyester resin B-1], 50 parts of the [master batch 1](pigment), and 2 parts of the [ketimine compound 1]. The resultant mixture was mixed by means of a TK Homomixer (manufactured by PRIMIX Corporation) at 5,000 rpm for 60 minutes, to thereby obtain [oil phase 1].

Note that, the above amounts are amounts of the solid contents of the materials.

<Synthesis of Organic Particle Emulsion (Particle Dispersion Liquid)>

A reaction vessel equipped with a stirring bar and a thermometer was charged with 683 parts of water, 11 parts of a sodium salt of sulfuric acid ester of methacrylic acid-ethylene oxide adduct (ELEMINOL RS-30, manufactured by Sanyo Chemical Industries, Ltd.), 138 parts of styrene, 138 parts of methacrylic acid, and 1 part of ammonium persulfate, and the resulting mixture was stirred for 15 minutes at 400 rpm, to thereby obtain a white emulsion. The obtained emulsion was heated to have the system temperature of 75° C., and was then allowed to react for 5 hours. To the resultant, 30 parts of a 1% ammonium persulfate aqueous solution was added, followed by aging for 5 hours at 75° C., to thereby obtain an aqueous dispersion liquid of a vinyl resin (a copolymer of styrene/methacrylic acid/sodium salt of sulfuric acid ester of methacrylic acid/ethylene oxide adduct), i.e., [particle dispersion liquid 1].

The [particle dispersion liquid 1] was measured by means of LA-920 (manufactured by HORIBA, Ltd.), and as a result, the volume average particle diameter thereof was found to be 0.14 µm. Part of the [particle dispersion liquid 1] was dried, and a resin component thereof was isolated.

<Preparation of Aqueous Phase>

Water (990 parts), 83 parts of the [particle dispersion liquid 1], 37 parts of a 48.5% aqueous solution of sodium dodecyldiphenyl ether disulfonate (ELEMINOL MON-7, manufactured by Sanyo Chemical Industries Ltd.), and 90 parts of ethyl acetate were mixed and stirred, to thereby obtain an opaque white liquid. The obtained liquid was used as [aqueous phase 1].

<Emulsification and Removal of Solvent>

To a container charged with the [oil phase 1], 1,200 parts of the [aqueous phase 1] was added, and the resulting mixture was mixed by means of a TK Homomixer at 13,000 rpm for 20 minutes, to thereby obtain [emulsified slurry 1].

A container equipped with a stirrer and a thermometer was charged with the [emulsified slurry 1], followed by removing the solvent therein at 30° C. for 8 hours. Thereafter, the resultant was matured at 45° C. for 4 hours, to thereby obtain [dispersion slurry 1].

<Washing and Drying>

After subjecting 100 parts of the [dispersion slurry] to filtration under the reduced pressure, the resultant was subjected twice to a series of treatments (1) to (4) described below, to thereby produce [filtration cake 1]:

46

(1): ion-exchanged water (100 parts) was added to the filtration cake, followed by mixing with TK Homomixer (at 12,000 rpm for 10 minutes) and then filtration;

(2): 10% aqueous sodium hydroxide solution (100 parts) was added to the filtration cake obtained in (1), followed by mixing with TK Homomixer (at 12,000 rpm for 30 minutes) and then filtration under reduced pressure;

(3): 10% by mass hydrochloric acid (100 parts) was added to the filtration cake obtained in (2), followed by mixing with TK Homomixer (at 12,000 rpm for 10 minutes) and then filtration; and

(4): ion-exchanged water (300 parts) was added to the filtration cake obtained in (3), followed by mixing with TK Homomixer (at 12,000 rpm for 10 minutes) and then filtration.

The [filtration cake 1] was dried with an air-circulating drier at 45° C. for 48 hours, and then was caused to pass through a sieve with a mesh size of 75 µm, to thereby prepare [toner 1].

Example 2

[Toner 2] was obtained in the same manner as in Example 1 except that the amount of the non-crystalline polyester resin A-1 was changed to 120 parts and the amount of the non-crystalline polyester resin B-1 was changed to 780 parts in the <Preparation of oil phase>.

Example 3

[Toner 3] was obtained in the same manner as in Example 1 except that the amount of the non-crystalline polyester resin A-1 was changed to 180 parts and the amount of the non-crystalline polyester resin B-1 was changed to 720 parts in the <Preparation of oil phase>.

Example 4

[Toner 4] was obtained in the same manner as in Example 1 except that the non-crystalline polyester resin A-1 was changed to the non-crystalline polyester resin A-2 and the non-crystalline polyester resin B-1 was changed to the non-crystalline polyester resin B-3.

Example 5

[Toner 5] was obtained in the same manner as in Example 1 except that the amount of the non-crystalline polyester resin A-1 was changed to 120 parts, the amount of the non-crystalline polyester resin B-1 was changed to 820 parts, and the amount of the crystalline polyester resin C-1 was changed to 10 parts in the <Preparation of oil phase>.

Example 6

[Toner 6] was obtained in the same manner as in Example 1 except that the amount of the non-crystalline polyester resin A-1 was changed to 180 parts and the amount of the crystalline polyester resin C-1 was changed to 20 parts in the <Preparation of oil phase>.

Example 7

[Toner 7] was obtained in the same manner as in Example 1 except that the non-crystalline polyester resin A-1 and the amount thereof were changed respectively to the non-crystalline polyester resin A-2 and 180 parts, and the non-

crystalline polyester resin B-1 and the amount thereof were changed respectively to the non-crystalline polyester resin B-3 and 720 parts.

## Example 8

[Toner 8] was obtained in the same manner as in Example 1 except that the amount of the non-crystalline polyester resin A-1 was changed to 120 parts, and the non-crystalline polyester resin B-1 and the amount thereof were changed respectively to the non-crystalline polyester resin B-2 and 780 parts in the <Preparation of oil phase>.

## Example 9

[Toner 9] was obtained in the same manner as in Example 1 except that the non-crystalline polyester resin A-1 was changed to the non-crystalline polyester resin A-2.

## Example 10

[Toner 10] was obtained in the same manner as in Example 1 except that the non-crystalline polyester resin B-1 was changed to the non-crystalline polyester resin B-2.

## Comparative Example 1

[Toner 11] was obtained in the same manner as in Example 1 except that the non-crystalline polyester resin A-1 was changed to the non-crystalline polyester resin A-5 and the non-crystalline polyester resin B-1 was changed to the non-crystalline polyester resin B-4 in the <Preparation of oil phase>.

## Comparative Example 2

[Toner 12] was obtained in the same manner as in Example 1 except that the non-crystalline polyester resin A-1 was changed to the non-crystalline polyester resin A-5 and the non-crystalline polyester resin B-1 was changed to the non-crystalline polyester resin B-5 in the <Preparation of oil phase>.

## Comparative Example 3

[Toner 13] was obtained in the same manner as in Example 1 except that the non-crystalline polyester resin A-1 was changed to the non-crystalline polyester resin A-3

and the non-crystalline polyester resin B-1 was changed to the non-crystalline polyester resin B-2 in the <Preparation of oil phase>.

## Comparative Example 4

[Toner 14] was obtained in the same manner as in Example 1 except that the non-crystalline polyester resin A-1 was changed to the non-crystalline polyester resin A-4, the non-crystalline polyester resin B-1 was changed to the non-crystalline polyester resin B-3, and the crystalline polyester resin C-1 was not used in the <Preparation of oil phase>.

## Comparative Example 5

[Toner 15] was obtained in the same manner as in Example 1 except that the non-crystalline polyester resin A-1 was changed to the non-crystalline polyester resin A-6 and the non-crystalline polyester resin B-1 was changed to the non-crystalline polyester resin B-4 in the <Preparation of oil phase>.

## Comparative Example 6

[Toner 16] was obtained in the same manner as in Example 1 except that the non-crystalline polyester resin A-1 was changed to the non-crystalline polyester resin A-6 and the non-crystalline polyester resin B-1 was changed to the non-crystalline polyester resin B-5 in the <Preparation of oil phase>.

## Comparative Example 7

[Toner 17] was obtained in the same manner as in Example 1 except that the amount of the non-crystalline polyester resin A-1 was changed to 50 parts and the amount of the non-crystalline polyester resin B-1 was changed to 850 parts in the <Preparation of oil phase>.

## Comparative Example 8

[Toner 18] was obtained in the same manner as in Example 1 except that the amount of the non-crystalline polyester resin A-1 was changed to 750 parts and the amount of the non-crystalline polyester resin B-1 was changed to 150 parts in the <Preparation of oil phase>.

Compositional ratios of the obtained toners are shown in Table 1.

TABLE 1

| Toner       | Kind | Parts by mass (i.e., PBM) | Non-crystalline polyester resin A |     | Non-crystalline polyester resin B |     | Crystalline polyester resin C-1 | Releasing agent | Pigment | Curing agent | Tg 1st (° C.) | Tg 2nd (° C.) |
|-------------|------|---------------------------|-----------------------------------|-----|-----------------------------------|-----|---------------------------------|-----------------|---------|--------------|---------------|---------------|
|             |      |                           | Kind                              | PBM | Kind                              | PBM |                                 |                 |         |              |               |               |
| Ex. 1       | 1    | A-1                       |                                   | 150 | B-1                               | 750 | 50                              | 50              | 50      | 2            | 43            | 22            |
| Ex. 2       | 2    | A-1                       |                                   | 120 | B-1                               | 780 | 50                              | 50              | 50      | 2            | 45            | 25            |
| Ex. 3       | 3    | A-1                       |                                   | 180 | B-1                               | 720 | 50                              | 50              | 50      | 2            | 41            | 20            |
| Ex. 4       | 4    | A-2                       |                                   | 150 | B-3                               | 750 | 50                              | 50              | 50      | 2            | 35            | -2            |
| Ex. 5       | 5    | A-1                       |                                   | 120 | B-1                               | 820 | 10                              | 50              | 50      | 2            | 45            | 38            |
| Ex. 6       | 6    | A-1                       |                                   | 180 | B-3                               | 750 | 20                              | 50              | 50      | 2            | 42            | 30            |
| Ex. 7       | 7    | A-2                       |                                   | 180 | B-3                               | 720 | 50                              | 50              | 50      | 2            | 40            | 18            |
| Ex. 8       | 8    | A-1                       |                                   | 120 | B-2                               | 780 | 50                              | 50              | 50      | 2            | 44            | 26            |
| Ex. 9       | 9    | A-2                       |                                   | 150 | B-1                               | 750 | 50                              | 50              | 50      | 2            | 38            | 23            |
| Ex. 10      | 10   | A-1                       |                                   | 150 | B-2                               | 750 | 50                              | 50              | 50      | 2            | 41            | 20            |
| Comp. Ex. 1 | 11   | A-5                       |                                   | 150 | B-4                               | 750 | 50                              | 50              | 50      | 2            | 30            | 15            |

TABLE 1-continued

|             | Non-crystalline polyester resin A |      |                           | Non-crystalline polyester resin B |     |     | Crystalline polyester resin C-1 | Releasing agent | Pigment | Curing agent | Tg 1st (° C.) | Tg 2nd (° C.) |
|-------------|-----------------------------------|------|---------------------------|-----------------------------------|-----|-----|---------------------------------|-----------------|---------|--------------|---------------|---------------|
|             | Toner                             | Kind | Parts by mass (i.e., PBM) | Kind                              | PBM | PBM |                                 |                 |         |              |               |               |
| Comp. Ex. 2 | 12                                | A-5  | 150                       | B-5                               | 750 | 50  | 50                              | 50              | 2       | 33           | 16            |               |
| Comp. Ex. 3 | 13                                | A-3  | 150                       | B-2                               | 750 | 50  | 50                              | 50              | 2       | 53           | 31            |               |
| Comp. Ex. 4 | 14                                | A-4  | 150                       | B-3                               | 750 | —   | 50                              | 50              | 2       | 52           | 51            |               |
| Comp. Ex. 5 | 15                                | A-6  | 150                       | B-4                               | 750 | 50  | 50                              | 50              | 2       | 36           | 20            |               |
| Comp. Ex. 6 | 16                                | A-6  | 150                       | B-5                               | 750 | 50  | 50                              | 50              | 2       | 40           | 22            |               |
| Comp. Ex. 7 | 17                                | A-1  | 50                        | B-1                               | 850 | 50  | 50                              | 50              | 2       | 61           | 53            |               |
| Comp. Ex. 8 | 18                                | A-1  | 750                       | B-1                               | 150 | 50  | 50                              | 50              | 2       | -30          | -33           |               |

15

**-Soxhlet Extraction-**

Each (1 part) of the toners was added to 40 parts of tetrahydrofuran (THF) and the mixture was refluxed for 6 hours. Thereafter, insoluble components were made to sediment with a centrifugal device, to thereby be separated from a supernatant.

The insoluble components were dried at 40° C. for 20 hours to obtain THF insoluble matter.

The solvent was removed from the above-separated supernatant, followed by drying at 40° C. for 20 hours, to thereby obtain THF soluble matter.

Table 2 shows [Tg1st (toner)], [Tg2nd (THF insoluble matter)], [Tg2nd (toner)], [G'(100) (toner)], [Tg2nd (THF soluble matter)], [G'(100) (THF insoluble matter)], [[G'(40) (THF insoluble matter)]/[G'(100) (THF insoluble matter)]], and amounts of the THF insoluble matter of the obtained toners.

**<Evaluation>**

Each of the obtained toners was used to prepare developers by the following method, and the following evaluation was performed on the prepared developers. The results are shown in Table 3.

**<<Production of Developer>>****-Production of Carrier-**

To 100 parts of toluene, 100 parts of a silicone resin (organosilicone), 5 parts of  $\gamma$ -(2-aminoethyl)aminopropyltrimethoxy silane, and 10 parts of carbon black were added, and the resultant mixture was dispersed by means of a homomixer for 20 minutes, to thereby prepare a resin layer coating liquid. To surfaces of spherical magnetite particles having the average particle diameter of 50  $\mu\text{m}$  (1,000 parts), the resin layer coating liquid was applied by means of a fluidized bed coating device, to thereby prepare a carrier.

**<Production of Developer>**

By means of a ball mill, 5 parts by mass of the toner and 95 parts by mass of the carrier were mixed, to thereby produce a developer.

**<<Offset Resistance>>**

Each of the developers was charged into a unit of IMA-GIO MP C4300 (product of Ricoh Company, Ltd.) and a rectangular solid image of 2 cm×15 cm was formed on PPC paper sheets (Type 6000<70W>A4 long grain (product of Ricoh Company, Ltd.) so that the toner was deposited in an amount of 0.40 mg/cm<sup>2</sup>. In the formation of the images, the surface temperature of the fixing roller was changed, and whether offset, in which an image remaining after development of the solid image is fixed in other places than the intended places, occurred was observed to evaluate offset resistance. Note that, the lowest temperature at which no offset occurred is defined as a minimum fixing temperature.

**[Evaluation Criteria for Cold Offset]**

- A: lower than 110° C.  
 B: 110° C. or higher but lower than 120° C.  
 C: 120° C. or higher but lower than 130° C.  
 D: 130° C. or higher

**[Evaluation Criteria for Hot Offset]**

- A: 170° C. or higher  
 B: 160° C. or higher but lower than 170° C.  
 C: 150° C. or higher but lower than 160° C.  
 D: lower than 150° C.

**<Heat Resistant Storage Stability>**

Each of the toners was charged into a 50 mL-glass container, which was then left to stand in a thermostat bath of 50° C. for 24 hours, followed by cooling to 24° C. The thus-treated toner was measured for penetration degree according to the penetration test (JIS K2235-1991) and evaluated for heat resistant storage stability according to the following criteria.

**35 [Evaluation Criteria]**

- A: The penetration degree was 20 mm or greater  
 B: The penetration degree was 15 mm or greater but less than 25 mm.  
 C: The penetration degree was 10 mm or greater but less than 15 mm.  
 D: The penetration degree was less than 10 mm.

**<Glossiness>**

An apparatus provided by modifying a fixing portion of copier MF2200 (product of Ricoh Company, Ltd.) using a TEFLON (registered trademark) roller as a fixing roller was used to perform a copy test on sheets of Type 6200 paper (product of Ricoh Company, Ltd.). Specifically, the fixing temperature was set to a temperature of 20° C. + the minimum fixing temperature determined in the evaluation of the low temperature fixing ability, and the paper-feeding linear velocity was set to 120 mm/sec to 150 mm/sec, the surface pressure was set to 1.2 kgf/cm<sup>2</sup>, and the nip width was set to 3 mm. The image after the copy test was measured for 60-degree glossiness with glossmeter VG-7000 (product of NIPPON DENSHOKU INDUSTRIES Co., Ltd.).

**[Evaluation Criteria]**

- A: 30% or more  
 B: 25% or more but less than 30%  
 C: 20% or more but less than 25%  
 D: less than 20%

**<<High Temperature, High-Humidity Storage Stability>>**

Each (5 g) of the toners was stored under an environment of 40° C. and 70% RH for 2 weeks. After that, the toner was sieved on a metal mesh having an opening of 106  $\mu\text{m}$  for 5 minutes, and an amount of the toner on the metal mesh was measured and evaluated according to the following evaluation criteria.

## [Evaluation Criteria]

- A: The amount of the toner on the metal mesh was 0 mg  
 B: The amount of the toner on the metal mesh was more than 0 mg but less than 2 mg.  
 C: The amount of the toner on the metal mesh was 2 mg or more but less than 50 mg.  
 D: The amount of the toner on the metal mesh was 50 mg or more.

wherein the THF insoluble matter has a storage modulus at 100° C. [G'(100) (THF insoluble matter)] of  $1.0 \times 10^5$  Pa to  $1.0 \times 10^7$  Pa, and

5 wherein a ratio of a storage modulus of the THF insoluble matter at 40° C. [G'(40) (THF insoluble matter)] to the storage modulus of the THF insoluble matter at 100° C. [G'(100) (THF insoluble matter)], expressed by  $[[G'(40)$

TABLE 2

|             | Tg1st toner<br>(° C.) | Tg2nd<br>THF<br>insoluble<br>matter<br>(° C.) | Tg2nd<br>toner<br>(° C.) | G'(100)<br>Toner<br>(Pa) | Tg2nd<br>THF soluble<br>matter<br>(° C.) | G'(100)<br>THF<br>insoluble<br>matter<br>(Pa) | G'(40)/G'(100)<br>THF insoluble<br>matter | Amount of THF<br>insoluble<br>matter<br>(% by mass) |
|-------------|-----------------------|-----------------------------------------------|--------------------------|--------------------------|------------------------------------------|-----------------------------------------------|-------------------------------------------|-----------------------------------------------------|
| Ex. 1       | 43                    | 3                                             | 22                       | $7.0 \times 10^3$        | 30                                       | $5.0 \times 10^5$                             | $3.1 \times 10$                           | 23                                                  |
| Ex. 2       | 45                    | 5                                             | 25                       | $5.5 \times 10^3$        | 33                                       | $3.2 \times 10^6$                             | $3.5 \times 10$                           | 20                                                  |
| Ex. 3       | 41                    | 0                                             | 20                       | $9.5 \times 10^3$        | 28                                       | $3.8 \times 10^5$                             | $2.5 \times 10$                           | 25                                                  |
| Ex. 4       | 35                    | -7                                            | -2                       | $5.1 \times 10^3$        | 26                                       | $3.9 \times 10^5$                             | $2.3 \times 10$                           | 22                                                  |
| Ex. 5       | 45                    | 6                                             | 38                       | $4.8 \times 10^4$        | 35                                       | $4.8 \times 10^6$                             | $3.4 \times 10$                           | 20                                                  |
| Ex. 6       | 42                    | -1                                            | 30                       | $5.0 \times 10^4$        | 46                                       | $7.0 \times 10^6$                             | $3.3 \times 10$                           | 27                                                  |
| Ex. 7       | 40                    | -13                                           | 18                       | $2.5 \times 10^3$        | 27                                       | $2.8 \times 10^5$                             | $2.6 \times 10$                           | 21                                                  |
| Ex. 8       | 44                    | 6                                             | 26                       | $7.5 \times 10^4$        | 32                                       | $3.0 \times 10^6$                             | $3.4 \times 10$                           | 27                                                  |
| Ex. 9       | 38                    | -10                                           | 23                       | $5.5 \times 10^3$        | 28                                       | $4.8 \times 10^5$                             | $3.0 \times 10$                           | 22                                                  |
| Ex. 10      | 41                    | 4                                             | 20                       | $6.5 \times 10^3$        | 29                                       | $5.2 \times 10^5$                             | $3.3 \times 10$                           | 25                                                  |
| Comp. Ex. 1 | 30                    | -43                                           | 15                       | $8.2 \times 10^3$        | 33                                       | $7.5 \times 10^7$                             | $6.0 \times 10$                           | 23                                                  |
| Comp. Ex. 2 | 33                    | -45                                           | 16                       | $3.5 \times 10^4$        | 35                                       | $9.0 \times 10^7$                             | $7.0 \times 10$                           | 24                                                  |
| Comp. Ex. 3 | 53                    | 32                                            | 31                       | $6.5 \times 10^5$        | 42                                       | $8.5 \times 10^4$                             | $1.5 \times 10^2$                         | 12                                                  |
| Comp. Ex. 4 | 52                    | 35                                            | 51                       | $6.0 \times 10^5$        | 45                                       | $8.0 \times 10^4$                             | $7.0 \times 10$                           | 36                                                  |
| Comp. Ex. 5 | 36                    | -41                                           | 20                       | $9.0 \times 10^3$        | 47                                       | $8.0 \times 10^7$                             | $6.5 \times 10$                           | 23                                                  |
| Comp. Ex. 6 | 40                    | -42                                           | 22                       | $2.5 \times 10^4$        | 50                                       | $9.8 \times 10^7$                             | $7.3 \times 10$                           | 22                                                  |
| Comp. Ex. 7 | 61                    | -38                                           | 53                       | $6.5 \times 10^2$        | 68                                       | $4.5 \times 10^5$                             | $3.2 \times 10$                           | 8                                                   |
| Comp. Ex. 8 | -30                   | -45                                           | -33                      | $3.5 \times 10^4$        | 52                                       | $2.5 \times 10^5$                             | $3.4 \times 10$                           | 72                                                  |

TABLE 3

|             | Cold<br>offset | Hot<br>offset | Heat resistant<br>storage stability | Glossi-<br>ness | High-temperature,<br>high-humidity<br>storage stability |
|-------------|----------------|---------------|-------------------------------------|-----------------|---------------------------------------------------------|
| Ex. 1       | A              | A             | A                                   | A               | A                                                       |
| Ex. 2       | B              | A             | B                                   | A               | A                                                       |
| Ex. 3       | A              | B             | B                                   | B               | A                                                       |
| Ex. 4       | A              | B             | C                                   | B               | C                                                       |
| Ex. 5       | C              | A             | A                                   | A               | B                                                       |
| Ex. 6       | C              | A             | A                                   | B               | B                                                       |
| Ex. 7       | C              | B             | B                                   | C               | B                                                       |
| Ex. 8       | C              | A             | B                                   | B               | B                                                       |
| Ex. 9       | A              | A             | A                                   | A               | B                                                       |
| Ex. 10      | A              | A             | A                                   | A               | A                                                       |
| Comp. Ex. 1 | A              | A             | A                                   | C               | D                                                       |
| Comp. Ex. 2 | A              | A             | A                                   | D               | D                                                       |
| Comp. Ex. 3 | D              | B             | A                                   | A               | A                                                       |
| Comp. Ex. 4 | D              | A             | A                                   | A               | A                                                       |
| Comp. Ex. 5 | A              | A             | A                                   | C               | D                                                       |
| Comp. Ex. 6 | A              | A             | A                                   | D               | D                                                       |
| Comp. Ex. 7 | D              | A             | A                                   | A               | A                                                       |
| Comp. Ex. 8 | A              | D             | D                                   | D               | D                                                       |

Embodiments of the present invention are as follows, for example.

<1> A toner,

wherein the toner has a glass transition temperature [Tg1st (toner)] of 20° C. to 50° C., where the glass transition temperature [Tg1st (toner)] is measured in a first heating in differential scanning calorimetry (DSC) of the toner,

wherein tetrahydrofuran (THF) insoluble matter of the toner has a glass transition temperature [Tg2nd (THF insoluble matter)] of -40° C. to 30° C., where the glass transition temperature [Tg2nd (THF insoluble matter)] is measured in a second heating in differential scanning calorimetry (DSC) of the THF insoluble matter,

(THF insoluble matter)]/[G'(100) (THF insoluble matter)]], is  $3.5 \times 10$  or less.

<2> The toner according to <1>, wherein the toner has a glass transition temperature [Tg2nd (toner)] of 0° C. to 30° C., where the glass transition temperature [Tg2nd (toner)] is measured in a second heating in differential scanning calorimetry (DSC) of the toner.

<3> The toner according to <1> or <2>, wherein a THF soluble matter of the toner has a glass transition temperature [Tg2nd (THF soluble matter)] of 5° C. to 35° C., where the glass transition temperature [Tg2nd (THF soluble matter)] is measured in a second heating in differential scanning calorimetry (DSC) of the THF soluble matter.

<4> The toner according to any one of <1> to <3>, wherein the toner has a storage modulus at 100° C. [G'(100) (toner)] of  $5.0 \times 10^3$  Pa to  $5.0 \times 10^4$  Pa.

<5> The toner according to any one of <1> to <4>, wherein the toner includes a non-crystalline polyester resin and a crystalline polyester resin as binder resins,

wherein the non-crystalline polyester resin includes a dicarboxylic acid component as a constituent component, and

55 wherein the dicarboxylic acid component includes terephthalic acid in an amount of 50 mol % or more.

<6> The toner according to any one of <1> to <4>, wherein the toner includes:

a crystalline polyester resin;

a non-crystalline polyester resin that contains a urethane bond, a urea bond, or both; and

a non-crystalline polyester resin that does not contain a urethane bond or a urea bond.

<7> The toner according to any one of <1> to <6>, wherein an amount of the THF insoluble matter in the toner is 15% by mass to 35% by mass.

## 53

<8> The toner according to any one of <1> to <7>, wherein the THF insoluble matter has a storage modulus at 100° C. [G'(100) (THF insoluble matter)] of  $5.0 \times 10^5$  Pa to  $5.0 \times 10^6$  Pa.

<9> A developer, including:

the toner according to any one of <1> to <8>; and a carrier.

<10> An image forming apparatus, including:

an electrostatic latent image bearing member; an electrostatic latent image forming unit configured to form an electrostatic latent image on the electrostatic latent image bearing member; and

a developing unit containing a toner and configured to develop the electrostatic latent image formed on the electrostatic latent image bearing member to form a visible image,

wherein the toner is the toner according to any one of <1> to <8>.

The invention claimed is:

1. A toner, comprising:

a binder resin; and tetrahydrofuran insoluble matter,

wherein the toner has a glass transition temperature Tg1st of 20° C. to 50° C., where the glass transition temperature Tg1st is measured in a first heating in differential scanning calorimetry of the toner,

wherein the tetrahydrofuran insoluble matter of the toner has a glass transition temperature Tg2nd of -40° C. to 30° C., where the glass transition temperature Tg2nd is measured in a second heating in differential scanning calorimetry of the tetrahydrofuran insoluble matter, wherein the tetrahydrofuran insoluble matter has a storage modulus at 100° C. of  $1.0 \times 10^5$  Pa to  $1.0 \times 10^7$  Pa, and wherein a ratio of a storage modulus of the tetrahydrofuran insoluble matter at 40° C. to the storage modulus of the tetrahydrofuran insoluble matter at 100° C. is  $3.5 \times 10$  or less.

2. The toner according to claim 1, wherein the toner has a second glass transition temperature of 0° C. to 30° C., as measured in a second heating in differential scanning calorimetry of the toner.

## 54

3. The toner according to claim 1, wherein a tetrahydrofuran soluble matter of the toner has a glass transition temperature of 5° C. to 35° C., as measured in a second heating in differential scanning calorimetry of the tetrahydrofuran soluble matter.

4. The toner according to claim 1, wherein the toner has a storage modulus at 100° C. of  $5.0 \times 10^3$  Pa to  $5.0 \times 10^4$  Pa.

5. The toner according to claim 1,

wherein the toner comprises a non-crystalline polyester resin and a crystalline polyester resin as binder resins, wherein the non-crystalline polyester resin comprises a dicarboxylic acid component as a constituent component, and

wherein the dicarboxylic acid component comprises terephthalic acid in an amount of 50 mol % or more.

6. The toner according to claim 1, wherein the toner comprises:

a crystalline polyester resin;

a non-crystalline polyester resin comprising a urethane bond, a urea bond, or both; and

a non-crystalline polyester resin that does not comprise a urethane bond or a urea bond.

7. The toner according to claim 1, wherein an amount of the tetrahydrofuran insoluble matter in the toner is 15% by mass to 35% by mass.

8. The toner according to claim 1, wherein the tetrahydrofuran insoluble matter has a storage modulus at 100° C. of  $5.0 \times 10^5$  Pa to  $5.0 \times 10^6$  Pa.

9. A developer, comprising:

the toner according to claim 1; and a carrier.

10. An image forming apparatus, comprising:

an electrostatic latent image bearing member; an electrostatic latent image forming unit configured to form an electrostatic latent image on the electrostatic latent image bearing member; and

a developing unit containing a toner and configured to develop the electrostatic latent image formed on the electrostatic latent image bearing member to form a visible image,

wherein the toner is the toner according to claim 1.

\* \* \* \* \*